# EUROPEAN PATENT SPECIFICATION

(11) **EP 1 927 997 B1**
(45) Date of publication and mention of the grant of the patent: **29.07.2009**
(21) Application number: 07254656.7
(22) Date of filing: 30.11.2007
(51) Int. Cl.: G21F 9/28, G21F 9/32

(54) **Steam reforming process system for graphite destruction and capture of radionuclides**
Dampfreformierungsverfahrenssystem für Graphitzerstörung und Erfassung von Radionukliden
Système de processus de reformage à la vapeur pour destruction graphite et capture de radionucléides

(30) Priority: 01.12.2006 US 872164 P; 09.11.2007 US 937650
(43) Date of publication of application: 04.06.2008
(73) Proprietor: Studsvik, Inc., Tennessee 37650 (US)
(72) Inventor: Mason, J.Bradley, Pasco, Washington 99301 (US)
(74) Representative: Howick, Nicholas Keith

(56) References cited:
- GB-A- 2 359 923
- GB-A- 2 381 649

## Description

### BACKGROUND OF THE INVENTION:

Graphite, which consists predominantly of the element carbon, is used as a moderator in a number of nuclear reactor designs, such as the MAGNOX and AGR gas cooled reactors in the United Kingdom, and the RBMK design in Russia. During construction, the moderator of the reactor is usually installed as an interlocking structure of graphite bricks. At the end of reactor life, the graphite moderator, typically weighing about 2,000 tons, is a form of radioactive waste which requires safe disposal.

Graphite is a relatively stable chemical form of carbon, which is in many ways suitable for direct disposal without processing. However, after neutron irradiation, the graphite will contain stored Wigner energy. The potential for release of this energy needs to be accommodated in any strategy which relies on disposing of the graphite in unprocessed form. Alternatively, processing the graphite before disposal can allow the safe release of any stored Wigner energy.

The graphite also contains significant quantities of radionuclides from neutron induced reactions, both in the graphite itself and in the minor impurities which it contains. Because of the structure of graphite, which includes loosely packed foliates or layers, the radioisotopes can become trapped within the spaces or pores of the graphite. The radioisotope content can conveniently be divided into two categories - short-lived isotopes and long-lived isotopes. Short-lived isotopes (such as cobalt-60) make the graphite difficult to handle immediately after reactor shutdown, but they decay after a few tens of years. Long-lived isotopes (principally carbon-14) are of concern through the possibility of their discharge to the biosphere. Processing the graphite offers the opportunity to separate the majority of the graphite mass (carbon) from the short-lived radioisotopes. This in turn facilitates disposal of the graphite waste shortly after the end of the reactor life, and may permit recycling.

Because of the characteristics of graphite and its mass, the most common procedure to date for decommissioning of graphite moderated reactors is to store the reactor core in-situ for a period of tens of years following reactor shut-down. During this period, short-lived radioisotopes decay sufficiently to allow eventual manual dismantling of the graphite moderator. Most plans then assume that the graphite will be disposed of in its existing chemical form, with appropriate additional packaging to prevent degradation or release over the long period of carbon-14 decay.

Storage has certain negative consequences, such as the following: 1) an implication of long-term financial liability, 2) a visually intrusive storage structure that has no productive purpose, and 3) a requirement imposed on a future generation (which gained no benefit from the original asset) to complete eventual clearance. If the storage alternative is to be replaced by shorter term management, it is essential for the graphite to be processed in a safe and radiologically acceptable manner.

Thus, there remains a need for a better way to handle radioactively contaminated graphite than simply storing it.

### SUMMARY OF THE INVENTION:

The following presents a simplified summary of the invention in order to provide a basic understanding of some aspects of the invention as set out in the present claims. This summary is not an extensive overview of the invention. It is not intended to identify key or critical elements of the invention or to delineate the scope of the invention. Its sole purpose is to present some concepts of the invention in a simplified form as a prelude to the more detailed description that is presented later.

The present invention includes a method for the treatment and recycling of graphite containing radionuclides. Generally, the present invention includes a two stage method that employs a thermal roaster that is operatively connected to a steam reformer. In the first stage, radioactive graphite is roasted or heated to volatize a first amount of radionuclides contained in the graphite. In the second stage, the roasted graphite is reacted with steam or gases containing water vapor so that a second amount of radionuclides is removed. The present method also includes the step of processing the radionuclides to enable their disposal.

A feature of the present invention includes the use of a thermal roaster for heating the radioactive graphite prior to reacting the radioactive graphite in the steam reformer. This method provides for a better concentration of the radionuclides so that processing steps are made safer and more efficient and the final volume of radioactive waste that requires ultimate solid disposal is reduced. Furthermore, by removing a first portion of radionuclides, the steam reforming process of the invention also becomes more manageable as less radioactive materials will potentially be discharged as gases to the environment.

### BRIEF DESCRIPTION OF THE DRAWINGS:

In the drawings,

FIG. 1 is schematic illustration of a system for treating radioactive graphite according to a preferred embodiment of the present invention;

FIG. 2 is a front view of a thermal moving bed roaster used in treating radioactive graphite according to a preferred embodiment of the present invention;

FIG. 3 is a front view of a steam reformer used in treating radioactive graphite according to a preferred embodiment of the present invention;

FIG. 4A is a front view of a steam reformer used in treating radioactive graphite according to a first alternative embodiment of the present invention; and

FIG. 4B is a front view of a steam reformer used in treating radioactive graphite according to a second alternative embodiment of the present invention;

FIG. 4C is a front view of a steam reformer used in treating radioactive graphite according to a third alternative embodiment of the present invention;

FIG. 4D is a front view of a steam reformer used in treating radioactive graphite according to a fourth alternative embodiment of the present invention;

FIG. 4E is a front view of a steam reformer used in treating radioactive graphite according to a fifth alternative embodiment of the present invention.

### DETAILED DESCRIPTION OF THE PREFERRED EMBODIMENTS:

Unless otherwise indicated, numbers expressing quantities of ingredients, constituents, reaction conditions and so forth used in the specification and claims are to be understood as being modified by the term "about." Accordingly, unless indicated to the contrary, the numerical parameters set forth in the specification and attached claims are approximations that may vary depending upon the desired properties sought to be obtained by the subject matter presented herein. At the very least, and not as an attempt to limit the application of the doctrine of equivalents to the scope of the claims, each numerical parameter should at least be construed in light of the number of reported significant digits and by applying ordinary rounding techniques. Notwithstanding that the numerical ranges and parameters setting forth the broad scope of the subject matter presented herein are approximations, the numerical values set forth in the specific examples are reported as precisely as possible. Any numerical value, however, inherently contains certain errors necessarily resulting from the standard deviation found in their respective testing measurements.

The present invention is a process applied to graphite materials previously used as the moderator in the core of a thermal nuclear reactor and which are no longer required for this purpose. It also applies to any other graphite materials (fuel element sleeves, braces etc.) irradiated in the neutron flux of a nuclear reactor core.

In a preferred embodiment, the present invention provides a process including the following steps: (i) heating the radioactive graphite in a thermal roaster; (ii) removing a first amount of radionuclides; (iii) reacting the radioactive graphite with a reforming agent, such as superheated steam or gases containing water vapor, to form hydrogen, carbon monoxide and carbon dioxide; (iv) reacting the hydrogen and carbon monoxide from step (iii) with an oxidizing agent to form water and carbon dioxide; (v) removing a second amount of radionuclides; and (vi) processing of radioactive contaminants. Step (iii) is a type of process that is generally referred to in the art as "steam reforming". The reaction in step (iii) may be carried out with the addition of oxygen to the steam or gases containing water vapor to provide exothermic reaction energy for the process. The addition of oxygen also enables the temperature of the steam reforming reaction to be controlled. As used herein, the term "agent" refers to a substance that can bring about a chemical reaction. Among other radionuclides commonly present in this type of graphite, the process of the present invention can effectively remove and treat any H-3, Cl-36, C-14, Fe-55, and Co-60 present in the graphite, as well as other radionuclides.

The advantage of the process of the present invention that utilizes steam and oxygen for gasification of the graphite, as compared to the use of air or oxygen enriched air combustion of radioactive graphite, is that it can be carried out under appropriately controlled containment conditions. For example, the steam reformer process can use cylindrical pressure vessels that provide a higher level of confinement than typical box type combustion-fired incinerators. Even more important is that air-fired combustion of graphite releases a large amount of heat that requires the addition of significant inert cooling gases to the incinerator to achieve reasonable graphite throughputs, however, this is not practical as the introduction of more inert gases substantially increases the off-gas flow such that collection and separation of the volatile H-3, C-14, and Cl-36 from such a proportionately large off-gas volume requires a much higher collection efficiency as the radioactive gases will be diluted by the inert cooling gas and the nitrogen in the air combustor and the off-gas treatment systems must be typically 10 to 20 times larger than is needed for an equivalent steam reformer unit where the off-gas flow is mainly steam that can be readily condensed and recycled back to the process as steam. The steam reformer also has the very significant advantage that very high levels of energy provided by oxygen oxidation of the graphite will be adsorbed by the corresponding adsorption of energy by the endothermic steam reforming reactions of steam with graphite. Additionally, the use of a deep bed in the reformer allows introduction of water to directly cool and adsorb the net positive heat from the combined steam reforming and oxygen oxidation of the graphite in the bed. This results in a very high graphite gasification rate for a relatively compact and more easily shielded reformer. In summary, the loss of hazardous or radioactive materials in the off-gas is therefore reduced or even eliminated and the low volume of off-gas simplifies handling including the possibility of achieving substantially zero gaseous emissions. The treatment throughput rate is higher for a given size hardware and capital investment. Further, the process enables the Wigner energy stored in the radioactive graphite to be released in a controlled manner.

The present invention will be further described with reference to FIG. 1 of the accompanying drawings which is an overview flow diagram of one means **10** of carrying out the process of the present invention. Referring to the drawing, the radioactive graphite is prepared for introduction to the first stage of the system. First, bulk radioactive graphite is removed and retrieved from a nuclear reactor core by means for retrieval **12.** Retrieval means can include a number of typically used mechanical, hydraulic, pneumatic or other means. In one embodiment, the graphite is retrieved by mechanically or "dry" cutting the graphite from the nuclear core of the reactor. If this option is employed, preferably, a remotely operated mechanical "nibbler" or cutter is used to reduce the size of the retrieved graphite blocks so that smaller pieces of graphite can be transferred from the nuclear reactor core to the mechanical sizing unit. Once cut from the core, the graphite is transferred pneumatically, or by other means, through an enclosed transfer system. Past graphite removal efforts could also be employed that have involved manual or robotic removal of large blocks of graphite. These large blocks of graphite could be transferred to a treatment system sizing means. In an alternative embodiment, a water jet cutting technique is employed along with a water slurry transfer system to retrieve the graphite from the core and move the graphite to the mechanical sizing unit. Regardless of the particular means employed to retrieve the graphite from the nuclear core, the processing system of the present invention will be capable of handling a wide variety of sizes of graphite blocks and pieces.

Next, the retrieved graphite, which includes large blocks and randomly sized pieces, is sized by a mechanical sizing unit 14 enclosing a means for mechanical sizing 18 the graphite. The mechanical sizing unit can also employ a variety of means and features to facilitate the sizing of the graphite. In one embodiment, the mechanical sizing unit includes an airlock inlet storage hopper **16** for the introduction of large blocks of graphite or randomly sized pieces of graphite to a thermal roaster (MBR) **20** to initiate the first stage of the present invention. This storage hopper **16** is provided with argon, CO₂, nitrogen or other substantially inert blanket gas and means for reducing the size of the graphite pieces. Furthermore, the storage hopper **16** provides a holdup capacity to the present system.

In operation, the graphite pieces will pass through the CO₂ or nitrogen blanketed sizing means **18,** which is capable of reducing the size or sizing the graphite pieces to about less than 20 mm (less than ¾ inch) in size. This small size is desirable to enhance the volatization of loosely held radionuclides from the graphite. Preferably, the sizing means **18** is a customized jaw or a rotary crusher that is dimensioned to reduce the size of the graphite to <20 mm sized pieces while also reducing the potential production of fines. Additionally, the sizing means **18** can include the use of a water seal to seal the sizing means from the MBR **20.** Preferably, the sizing means **18** is operated at a low speed, about <100 rpm, that generates a low amount of fines, about <5%.

Once the graphite pieces have been sized, they are fed through a sealed lock-hopper **17** to the MBR **20** to undergo the first stage of the present system. In one embodiment, a means to use slurry transfer of retrieved graphite from the reactor core to the sizing means **18** can be used. Water will separate by gravity and seal the bottom of the sizing means **18** with solids being mechanically transferred from the bottom of the sizing means 18 to the sealed lock-hopper **17** to the MBR **20.** The MBR **20,** which is shown in more detail in FIG. 2 includes a refractory lined vessel **22** with an internal shell or liner **24** that can be preferably electrically heated. Preferably, the MBR **20** is dimensioned to contain approximately 24 hours of throughput of graphite. Additionally, the MBR **20** includes an inlet for the introduction of graphite and, optionally, a separate inlet for oxygen above the normal graphite levels in the side of the vessel **22,** as well as two outlets, **23** and **25,** one for outlet gases and fines exiting the MBR **20.** and one for roasted graphite, which can also serve as the inlet for purging gases.

The use of an electrically heated MBR **20** is a feature of the present invention, as electrical heat will eliminate the need to produce energy within the MBR, such as by the addition of oxygen, which would oxidize the graphite. Because a goal of the present invention is to volatize and remove an amount of radionuclides, including C-14, the oxidation of the graphite in the roaster to produce a carbon-oxide gas, including CO or CO₂, would dilute the very C-14 containing CO and CO₂ that is being separated and concentrated. A small amount of oxygen that is introduced occasionally or periodically, however, may be needed to help oxidize certain species of radionuclides in the pores of the graphite to enhance their mobility so that they can be removed from the graphite pores more readily.

Preferably, the graphite pieces are introduced from the sealed inlet lock-hopper **17** into the top of the MBR **20** so that the graphite can move from the top of the vessel **22** to the bottom in a continuous, or semi-continuous manner. Once the pieces are within the MBR vessel **22,** the temperature of the internal shell **24** is heated to an operating temperature of between about 400° to about 1200°C. The graphite bed moves downward through the slow semi-continuous removal of graphite out the bottom of the MBR **20.** Preferably, the operating temperature is between about 600° to about 1100°C, and most preferably it is between about 700° to about 1000°C. During this heating, the graphite pieces move slowly down the height of the MBR 20 and are removed from the bottom and thereafter transferred to a graphite gasification steam reformer (GGR) 50 to initiate the second stage of the present system.

Upon reaching a suitable operating temperature, the graphite is soaked or kept at this temperature to allow the volatile radioactive materials that are mechanically trapped in the spaces or pores of the graphite to migrate out of the graphite. The soaking time required to sufficiently volatize the radioactive materials on the surfaces and pores of the graphite is between about 2 to 36 hrs, with the preferred soaking time being between about 4 to 24 hrs, and the most preferred soaking time being between about 10 to 18 hrs. Depending on the particular radionuclides contained in the graphite, the roasting and soaking steps will facilitate the volatization and migration of C-14, H-3, and Cl-36. The C-14 takes two forms in graphite. There is C-14 as a component of CO2, which is produced from the neutron flux activation of nitrogen. The second is C-14 produced within the graphite structure from the activation of C-13. The C-14 produced from the activation of nitrogen can be diffused from the pores of the graphite through heating and purging. The remaining C-14 must be gasified. Preferably, about 40% to about 60% of the C-14, and a majority of the H-3 and Cl-36 trapped in the graphite is volatized and removed from the graphite during this stage of the system while preventing the gasification of the base graphite.

To further facilitate the volatization of radionuclides from the graphite, a small flow of purge gases, which can include both inert and reactive gases, is introduced to the bottom of the MBR so that the purge gases flow upwards as the graphite pieces move slowly downward. Inert purge gases include argon, nitrogen, and/or CO₂, and reactive purge gases include oxygen, oxygen containing gases like CO, and/or steam. Also, organic vapors that contain oxygen in the molecules, as well as inert gases such as CO₂, can be employed.

The countercurrent flow of purge gases enhances the volatization and diffusion of the radionuclides from the graphite although a co-current roaster can also be used. Because inert and/or reactive gases are introduced to the MBR 20, the radionuclides are carried out in a number of forms. In particular, if the graphite contains loosely held C-14, this will be volatized and carried out of the MBR as CO₂ gas. The C-14 will be converted to CO and CO₂ by the steam and/or oxygen that is introduced. The H-3 is reacted and volatized by the steam and/or oxygen to make H₂O or gaseous H₂. Furthermore, if H-3 gas is adsorbed in the graphite matrix, the purge gas flow can desorb this gas from the graphite. The Cl-36 is reacted and volatized by the purge gases to make HCl. Furthermore, if the Cl-36 is an adsorbed gas in the graphite matrix, it can also be volatized or desorbed by the purge gas flow. Other radionuclides (e.g., Co60, Fe55) that are not volatized or reacted remain in the graphite which proceeds to the second stage GGR **50.**

Preferably, the C-14 CO₂ is concentrated by a factor of up to 50X by the preferential volatization of much of C-14 without the equivalent gasification of the graphite. It is thus important to limit the level of oxidizing gas that is introduced to the MBR 20. Although a small amount of oxygen is useful in converting any CO formed by the steam reforming reactions between the graphite and the steam to CO₂, the gasification of the graphite is preferably limited to no more than about 2% to 4%. To ensure any CO within the unit is converted to CO₂, however, oxygen gas is also introduced at the top of the MBR 20.

This countercurrent flow of gases is further combined with pressure swings and/or vacuum swings in the MBR **20** to drive the gases in and out of the pores or spaces of the graphite to enhance otherwise slow diffusion of the volatized radionuclides from the graphite. If only vacuum swings are employed, these swings may be from about -200 inch WC to about -10 inch WC. If only pressure swings are employed, the pressure may be from about ambient to about 30 psig or even higher. Alternatively, both pressure and vacuum swings can be employed. Throughout the pressure/vacuum swings, the operating temperature will remain about the same, and the pressure/vacuum swings will be cycled over time with a cycle starting as soon as the previous one is completed. The preferred protocol for using temperature, pressure, and/or vacuum conditions in the MBR **20** will be based on analysis of radionuclides, which are specific for each graphite source, in parametric test runs that will determine the optimum removal efficiency (% removed) as a function of composition of purge gas, temperature, and pressure cycling speed and depth of pressure variation.

In a continuous or semi-continuous manner, roasted graphite will exit the MBR **20** from the bottom outlet **23,** and a gas stream containing a mixture of purge gases and volatized radionuclides will exit the MBR **20** from an upper outlet **25.** Processing steps relating to the radionuclide containing outlet gas stream will be discussed further below.

The roasted graphite will next enter the GGR **50** to undergo the second stage of the present system. The fine solids that carryover from the MBR **20** are collected in a roaster outlet gas filter (RGF) **800** and then transferred to the GGR **50.** The RGF **800** is a small filter that will contain a set of silicon carbide or sintered powdered metal filter elements for efficient removal of particulate in the MBR 20 outlet gas stream. The RGF **800** is optionally provided with a small sealed lock-hopper that will transfer the fine graphite solids to the GGR **50** by dilute or dense phase transfer using CO₂ as the transfer gas. Larger graphite solids are transferred from the bottom of the MBR **20** to the GGR **50.** In this context, the term "roasted" means that a portion of the volatile radionuclides contained within the graphite has been removed in the MBR **20.** The GGR **50** is a feature of the present invention, as it efficiently gasifies graphite while producing a minimum volume of process gases that require treatment. Destruction of the graphite is achieved in the GGR **50** through heating of the graphite at a temperature of about 800° to 1200°C, preferably 900° to 1100°C, in a steam and/or oxygen environment, which gasifies the graphite into CO₂ and CO. Generally, GGR 50 includes a vertical, refractory lined vessel that employs a fixed and/or fluid bed system and autothermal steam reforming conditions to gasify the graphite and release the remaining fraction of H-3, Cl-36 and C-14, as well as to separate non-volatile radionuclides (Co-60, Fe-55, etc.) that are also contained in the graphite structure. As used herein, "autothermal" refers to the internal heating conditions provided by the heated steam introduced to the vessel and/or high energy release from the graphite gasification to CO and CO₂.

A number of operation modes can be used to react the graphite within the GGR **50.** As shown in more detail in FIG. 3, a preferred embodiment of the GGR **50** includes a lower fixed bed 52 that includes larger pieces of graphite and an upper fluidized bed **54** that includes smaller pieces of graphite that are fluidized by fluidizing gases. As used herein, "fluidize" means to suspend or transport finely divided particles in a stream of gas or air. The particles of graphite in the fluidized bed **54** are such that when acted on by fluidizing gases, these particles act as a fluid in a generally bubbling bed mode. At the lower portion of the fixed bed **52,** the GGR **50** includes water and oxygen jets **56** and/or a steam and fluidizing gas inlet **58.** Oxygen can also be introduced at or above the fluidized bed **54** so as to ensure that any CO produced within the GGR **50** is converted to CO₂. The fluidizing gases typically include steam or steam and oxygen although other fluidizing gases can be used such as nitrogen, carbon dioxide, and other oxygen-containing or inert gases. The term "fixed bed" refers to any bed of solid particles that are not fully fluidized and includes a slowly moving bed of solids that generally move downward over time, as well as non-continuous or partially fluidized beds.

To initiate the reforming reactions, heated steam from a boiler **300** is introduced to the lower portion of the fixed bed **52.** Because the graphite in the GGR **50** is heated and reacted at the lower portion of the fixed bed **52,** the graphite particles in this area of the GGR **50** will shrink in size as the gasification or reforming products (CO and H₂) rise up through the voids between the larger fixed bed **52** graphite particles. Thereafter, the larger particles will migrate or settle to the bottom to take the place of the smaller particles similar to the larger graphite particles in the MBR **20.** The smaller graphite particles are more easily fluidized. Thus, as the graphite is being reformed, the fluidized bed **54** continues to grow and the fixed bed **52** continues to shrink in size. The settling of the larger particles is further facilitated through the use of the water oxygen jet **56,** which provides agitation to localized areas within the generally fixed bed **52** particles.

In a first alternative embodiment shown in FIG. 4A, the GGR **60** includes only a fixed bed **62.** At the lower portion of the fixed bed **62,** the GGR **60** includes a water and oxygen jet 66 and/or a steam and fluidizing gas inlet **68.** Oxygen can also be introduced at or above the top portion of the fixed bed **62** so as to ensure that any CO produced within the GGR **60** is converted to CO₂. This operation mode may be preferred from an energy standpoint if the gas flows employed are very low such that the smaller particles produced in the bottom of the fixed bed **62** are not carried out as fines and are consumed within the bed, hence there is substantially no fluidized bed above the fixed bed.

In a second alternative embodiment shown in FIG. **4B****,** the GGR **70** includes only a fluidized bed **74,** also referred to as a "bubbling" bed. At the lower portion of the fluidized bed **74,** the GGR 70 includes a water and oxygen jet **76** and/or a steam and fluidizing gas inlet **78.** Oxygen can also be introduced at or above the top portion of the fluidized bed **74** so as to ensure that any CO produced within the GGR **70** is converted to CO₂. This operation mode may be preferred from an efficiency standpoint if the graphite particles being gasified and reformed are small enough to become fluidized.

The third alternative embodiment shown in FIG. 4C is nearly identical to the second alternative embodiment shown in FIG. 4B, except that a water and oxygen jet is missing. The GGR **80** includes only a fluidized bed **84,** also referred to as a "bubbling" bed. At the lower portion of the fluidized bed **84,** the GGR **80** includes a steam and fluidizing gas inlet **88.** Oxygen can also be introduced at or above the top portion of the fluidized bed **84** so as to ensure that any CO produced within the GGR **80** is converted to CO₂.

In a fourth alternative embodiment shown in FIG. 4D, the GGR **90** includes a spouted bed **91** that is formed by a water and oxygen jet **98** or a steam and oxygen jet (not shown) that is introduced to the bottom of the vessel so that a spout entirely penetrates a fixed bed **92** of graphite particles. Oxygen can also be introduced at or above the top portion of the spouted bed **91** so as to ensure that any CO produced within the GGR **90** is converted to CO₂. This may be preferred from an efficiency standpoint.

In a fifth alternative embodiment shown in FIG. 4E, the GGR **100** includes a partially spouted lower bed **101** and an upper fluidized bed **104.** At the lower portion of the partially spouted bed is also included a steam and fluidizing gas inlet **68.** The partially spouted bed **101** is formed by a water and oxygen jet **108** (or a steam and oxygen jet (not shown)) that is introduced to the bottom of the vessel so that a spout partially penetrates a fixed bed **102** of graphite particles. Oxygen can also be introduced at or above the top portion of the fluidized bed **104** so as to ensure that any CO produced within the GGR **100** is converted to CO₂. This may be preferred from an efficiency standpoint.

Although the operation modes of the GGR **50** can vary, the inorganic ash from the gasification of the graphite and gases formed from steam reforming and oxidizing reactions are processed similarly. The inorganic ash, including the non-volatile radionuclides, is converted into small granules by the introduction of an additive in the GGR **50** that mineralizes the metals and metal oxides in the ash into stable non-volatile spinels and minerals, generally fine particulates. The elutriated fine graphite and ash particles and reformed gases are sent to a graphite gasification cooler (GGC) **202.** The inorganic residues from the steam reforming reactions are largely removed by the GGC **202** with the balance being removed by a graphite gasification filter (GGF) **206.** The removed ash, as well as metal oxides, and metal spinel particles are transferred as a slurry to an optional slurry concentrator filter (SCF) **600,** described further below, and then to a solidification unit **500** where they are solidified into a cement matrix for disposal as solid waste **502.**

More specifically, reformed gases (mainly steam and CO₂) and elutriated graphite and ash fines exit the GGR **50** at line **200** and enter the GGC **202,** which is a venturi scrubber/condenser/cooler that quenches and cools the high temperature gases to the steam saturation temperature of the process. Cooling in the GGC is provided by an external closed loop chiller system. The GGC **202** is provided with an integral wet scrubber to remove any Cl-36 as a salt with the addition of caustic materials (e.g., NaOH or similarly basic materials) and to remove fine graphite particles in the GGR outlet gas for recycle to the GGR **50.**

After entering the GGC **202,** the fine graphite particles are returned to the GGR 50 as a water/graphite slurry through line **204** for gasification. Oxygen is used to atomize the water/graphite fines slurry into the GGR **50** to improve the efficiency of fine graphite gasification that is problematic in other types of thermal treatment systems. As solids accumulate in the GGC **202,** a portion of the solids is transferred to the slurry concentrator filter (SCF) **600,** where graphite fines are removed from the more dense metal oxides, metal spinels and mineralized ash particulates. In particular, the SCF **600** includes a small settling/filtration unit that is dimensioned to differentially separate graphite fines from other insolubles in the water stream from the GGC **202** and a roaster condenser scrubber (RCS) **700** that will be described in more detail below. The non-graphite insolubles produced in the process include: inorganic ash constituents and non-volatile radionuclides that are in granular form as spinels, metal oxides, fused ashes, and other mineral forms. These insolubles are heavier than the very fine graphite particles and can be reasonably separated using nuclearized versions of standard industrial equipment. "Nuclearized" means that versions of standard industrial equipment are modified to provide suitable levels of radiation shielding and to facilitate remote maintenance and cleaning after use. The non-graphite insolubles and some of the water and dissolved solids are periodically removed from the SCF **600** and transferred to the solidification unit 500, where they are solidified into stable monoliths. Essentially all the H-3 as water and all non-volatile radionuclides are thereby made into stable solid matrices for disposal as a solid waste. Since the gamma producing radionuclides, mainly Co-60 and Fe-55, are concentrated into a small volume waste form, the SCF 600 and the solidification unit **500** require shielding. A portion of the filtered water is separated in the SCF **600** and is pumped to the boiler 300, thereby recycling the process water ultimately to the MBR **20** and the GGR **50** as steam. This recycle of process water serves to concentrate salts, such as the low concentration Cl-36, in the boiler **300** blowdown that is generally directly discharged as a liquid waste or optionally input to the solidification unit **500** as the water source for preparing the solidification matrix.

A feature of the present invention includes the use of a GGR **50** that can accommodate a high concentration of graphite fines that are almost impossible to handle and gasify in an air combustion-fired incineration unit. The recycle of the graphite fines in a water slurry from the GGC **202** to the GGR **50** is atomized with oxygen-containing gases into the bottom of the GGR 50 ensures that graphite fines will be efficiently gasified with good temperature control. The input of liquid water serves as a very effective, high capacity heat sink for the process as a result of autothermal energy generation from exothermic oxidizing reaction of oxygen and the fine graphite particles. The upper section of the GGR **50** operates with a separate injection of oxygen to convert any CO and hydrogen to CO₂ and water vapor so that no downstream oxidizer is required.

The steam cooled and condensed by the GGC **202** is also reused or further processed. For example, the steam and the balance of H-3 that is volatized as water vapor can be condensed for reuse as cooling water in the GGR **50** and for the makeup of water to feed the boiler **300,** which provides heated steam to the GGR **50** and MBR 20. Furthermore, the high energy released from the graphite gasification to CO₂ can be adsorbed by the injection of water slurry from the GGC **202.** The water/fines slurry is atomized into the GGR by a metered quantity of oxygen-containing gas 220. Through the use of evaporation of the water the temperature of the GGR **50** is more easily controlled so as to prevent certain radionuclides from volatizing, such as Co-60 and Fe-55. The use of direct water injection with oxygen-containing gas atomization will also provide for high throughputs in a relatively small reformer unit.

The cooled low moisture gas stream exiting the GGC **202** is preferably double filtered through the GGF **206** to remove any non-volatile radionuclides and any remaining fine graphite particles from the gas stream. Preferably, the GGF **206** is a pulse-back filter vessel with sets of sintered metal filter elements that are designed to remove >99.95% of particulates smaller than 0.3 micron. The GGF **206** filter media is periodically cleaned by means of pressurized CO₂. The GGF is followed by a HEPA filter with bag-in and bag-out capability.

The fines removed by the GGF **206** are returned to the GGC **202** through line **230** where the particulates are mixed with the condensed water in the GGC **202** and thereafter returned to the GGR **50** as a water/graphite fines slurry through line **204.** Alternatively, the GGF **206** is provided with a small sealed lock-hopper that will transfer the fine graphite solids directly to the GGR **50** by dilute phase transfer using CO₂ as the transfer gas. The filtered gas stream is then passed through a moisture adsorber 208 where residual moisture and final traces of H-3 water are removed from the gas stream.

The moisture adsorber **208** is preferably a vessel that contains a regenerable bed of adsorption media that is designed to remove residual water vapor from the gas stream. The removal of the residual water vapor will ensure that essentially all of the H-3 water is removed from the gas stream before the gas is discharged into the environment. The water that is collected from the regenerable adsorption media is recycled back to the boiler **300** to provide a source of water.

Accordingly, the boiler **300** of the present invention receives water from a number of sources within the present system. The boiler **300** is preferably a customized electrically heated steam generator that receives filtered water from the RCS **700,** described below, and the GGC **202** after being filtered in the SCF **600.** The boiler **300** employs a special alloy construction to provide the required steam for use in the MBR **20** and the GGR **50.** Dissolved solids, such as Cl-36 and soluble ash constituents in the graphite are concentrated in the boiler **300.** Further, the pH of the water in the boiler 300 is adjusted with caustic addition to keep the pH preferably between 6 and 10.

When dissolved solids in the boiler water reach the maximum desired solids concentration, the boiler **300** is blown down, meaning that a portion of this water with dissolved solids is removed from the boiler **300.** The boiler blow-down water can be either directly discharged as a liquid or the small volume of blow-down can be solidified into a cement matrix. The majority of the Cl-36 will be in this blow-down water as sodium chloride or alternative salt or mineral.

If the release of Cl-36 as a liquid or solidified matrix is unacceptable due to the high mobility of Cl-36 in the disposal facility, an optional small scale pyrolysis mineralizer evaporator could be added to process the boiler blow-down into a stable, water insoluble mineral monolith. The pyrolysis/mineralizer is an electrically heated drum-sized thermal treatment unit. Clay is mixed with the boiler blow-down and the water/clay slurry with dissolved salts are sprayed or injected into the pyrolysis/mineralizer where the salts are converted into water insoluble alumino-silicate minerals in a monolithic form. The Cl-36 NaCl is preferably converted to a water insoluble mineral called Sodalite, Na₆[Al₂O₃-2SiO₂]₆-2NaCl.

Upon exiting the moisture adsorber **208,** the dry gas stream, which is a low volume CO₂-rich gas with residual C-14 as CO₂, can then be directly discharged into the environment through a stack **402** or it can alternatively be converted to water soluble carbonates in an optional mineralization unit **400** and discharged as an aqueous soluble carbonate liquid. Alternatively, the C-14 CO₂ can be directly discharged as gas from the GGR **50.** The mineralization unit **400** can be a combination pyrolysis and mineralization unit. Alternatively, the graphite from the GGR **50** can be transported to the mineralization unit **400** and thereafter discharged as an aqueous soluble carbonate liquid. Additionally, the CO₂ could be liquefied by a CO₂ amine liquefaction unit such as made commercially available by the Wittemann Company, and described in US Patent No. 2,663,154, which is incorporated herein by reference. The concentrated CO₂ liquid could then be shipped to an alternative release/discharge point for vaporization and discharge as a low volume gas.

A feature of the present invention includes the use of low gas flows as compared with typical air combustion-fired incineration units. The use of steam in the GGR 50 allows for simple condensation of the water vapor to remove the bulk of the thermal process outlet gas stream flow leaving a mainly CO₂-rich gas stream for conversion to a soluble carbonate solution using the optional mineralization unit **400** or that is amenable to simple separation and liquefaction using small scale commercially available CO₂ recovery systems with the addition of the optional CO₂ liquefaction unit.

As previously discussed, the radionuclide containing outlet gas stream from the MBR 20 requires further processing prior to disposal or release into the environment. This additional processing can be achieved by a variety of optional methods or means. In one embodiment, the outlet gas stream is filtered through a downstream roaster gas filter (RGF) **800** to remove and collect any fine graphite particles that may be present in the gas stream. Any such collected solids will be transferred to the GGR **50** for the purpose of gasification of the particles. More specifically, the RGF **800** is a small, high temperature filter that contains a set of silicon carbide or sintered powdered metal filter elements. The RGF **800** is preferably provided with a small sealed lock-hopper that is connected to a transfer system, whereby fine graphite solids are transferred pneumatically by dilute phase transfer or dense phase transfer using CO₂ as the transfer gas.

Once filtered, the radionuclide containing gas stream is sent to a combined condenser and scrubber, referred to herein as the roaster condenser scrubber (RCS) **700,** which is used to condense the water vapor contained in the gas stream to remove H-3 as water, and the remaining gases are scrubbed with the condensed water solution to remove Cl-36 as salt. Alternatively, the radionuclide containing gas stream can be sent directly from the MBR **20** to the RCS **700** without the need for an upstream filter. In particular, the RCS 700 is a small sized wet scrubber that includes a chilled water recirculation system that is used to condense a majority of the water vapor in the outlet gas stream. The condenser water will adsorb substantially all of the amount of Cl-36 that was volatized in the roaster unit. The condensed water and collected Cl-36 will than be pumped to the SCF concentrator **600** previously described for removal of any undissolved solids in the solution. The partially cleaned water with traces of dissolved species, including the Cl-36, will then go to the boiler **300** to be used as a water source or otherwise disposed as boiler blow-down water, as previously described.

Optionally, the small amounts of non-condensable gases, such as carbon-oxide gases, and mainly CO₂-rich with both C-14 and C-12, resulting from the condensed and scrubbed outlet gas stream are passed through a CO₂ liquefaction system **900.** As used herein, the term "carbon-oxide" can include CO and CO₂ and is interchangeable with CO and CO₂. This CO₂ liquefaction system removes, concentrates and liquefies the carbon-oxide, including C-14 carbon dioxide, for remote discharge or for further treatment to concentrate the C-14 in a CO Converter **904** and a PSA C-14 Separator **906.** If further treatment through the CO Converter and Pressure Swing Adsorption (PSA) Separator is required, it is preferred to liquefy the CO₂ for ease of storage and so that the cyclical gas flows from the MBR 20 will not impact the operation of the CO Converter **904** and the PSA Separator **906,** which both require a stable gas flow for optimal performance. The liquefied CO₂ is therefore vaporized as required to meet the process flow requirements of the CO Converter **904** and PSA Separator **906.**

In one embodiment, the CO₂ liquefaction system is a small capacity unit that includes a simple chilled condenser **902** that condenses CO₂ as liquid or solid. In an alternative embodiment CO₂ liquefaction unit is a small capacity unit that includes an amine based CO₂ recovery and liquefaction system, such as the liquefaction system made commercially available by the Wittemann Company as previously described. There exist a number of other commercially available systems that are suitable for the liquefaction of CO₂.

Once the CO₂ is liquefied, the CO₂ is optionally sent to the CO Converter **904** that includes a catalytic fixed bed for the conversion of CO₂ to CO gas. The CO₂ must be vaporized prior to entry into the CO Converter **904.** This CO gas is then passed through the PSA C-14 separator **906** for the separation of C-14 CO from C-12 CO. If the PSA Separator **906** is to be used in the flow path, oxygen can be omitted from the top of the MBR **20** to maximize the CO content of the MBR 20 outlet gases to thereby minimize the load on the CO Converter **904.** The PSA separator 906 includes several, automated adsorption columns that are filled with a special zeolite media. In operation, the CO gas passes through the zeolite adsorption columns at a controlled temperature and pressure so that substantially all of the CO (both C-12 and C-14 forms) is adsorbed on the zeolite. The process flow is then reversed and the pressure adjusted such that the C-14 carbon monoxide is preferentially released by the zeolite. Through the utilization of multiple separation steps, a higher purity of C-14 based carbon monoxide can be achieved. This C-14 enriched carbon monoxide can then be incorporated into a carbonate or silicon carbide solid matrix for final disposal of the concentrated C-14 waste. Preferably, the C-14 enriched CO is converted to C-14 enriched carbon-oxide which can then be converted to a carbonate or carbide form. Alternatively, The C-14 enriched CO stream from the PSA Separator can be converted to C-14 CO₂ and can be optionally sold and further purified if necessary for beneficial reuse as C-14 in the medical or scientific fields.

The use of a PSA C-14 separator **906** is a feature of the present invention. Through the use of this separator, about 40% to 60% of the total C-14 contained in the graphite can be concentrated and converted to a stable solid matrix that has 1 % to 5% of the final disposal volume of the graphite treated by the MBR **20.** This provides for maximum stability of the final C-14 products with minimal impact on disposal volumes.

As an alternative to the liquefaction of the CO₂ containing outlet gas stream exiting the RCS **700,** the gas stream can pass through the mineralization unit **400.** This unit is a wet scrubber that adsorbs the CO₂ present in the gas stream in an aqueous solution of caustic (NaOH, lime, or other basic materials) to form soluble carbonates or mineral forms that are then discharged as a liquid or solidified into a cement matrix. Thereafter, the cleaned and scrubbed gases from the mineralization unit **400,** which mainly include non-condensable gases having trace amounts of CO₂, are transferred to the moisture adsorber **208** where final traces of moisture are removed from the gas so as to also remove all traces of H-3 water from the gas stream. These cleaned non-condensable gases commingle with the offgases from the steam reformer and are discharged out of a common stack.

Those skilled in the art of steam reforming and graphite gasification systems will recognize that many substitutions and modifications can be made in the foregoing preferred embodiments without departing from the scope of the present invention.

## Claims

1. A method for graphite destruction and capture of radionuclides, comprising:
providing graphite containing radionuclides;
providing a roaster;
heating said graphite in said roaster;
removing a first amount of radionuclides from said graphite;
providing a steam reformer;
reacting said graphite with a reforming agent in said steam reformer to form a carbon oxide;
removing a second amount of radionuclides from said graphite;
processing said first amount and second amount of radionuclides.

2. The method as recited in claim 1, wherein said carbon oxide is carbon monoxide.

3. The method as recited in claim 2, further comprising:
reacting said carbon monoxide with an oxidizing agent in said steam reformer to form carbon dioxide.

4. The method as recited in claim 1, further comprising:
providing a sizing means that is operatively connected to said roaster; and
sizing said graphite with said sizing means.

5. The method as recited in claim 4, wherein said sizing means is a crusher dimensioned to reduce the size of said graphite to pieces that are about less than 20 mm, while also reducing the potential production of graphite fines.

6. The method as recited in claim 4, wherein said sizing means is operated at a low speed that generates a low amount of fines.

7. The method as recited in claim 6, wherein said low speed is about less than 100 rpm, and wherein said low amount is about less than 10%.

8. The method as recited in claim 6, wherein said low amount is about less than 5%.

9. The method as recited in claim 4, wherein said sizing means includes an inert gas blanket.

10. The method as recited in claim 9, wherein said inert gas blanket is made of one or more of the following, including argon, nitrogen, and CO₂.

11. The method as recited in claim 4, wherein said sizing means includes a water seal.

12. The method as recited in claim 11, further comprising the steps of providing means for slurry transfer and transferring said graphite from a reactor core to said sizing means.

13. The method as recited in claim 4, wherein said sizing means is highly pressurized water.

14. The method as recited in claim 1, wherein said first amount of radionuclides includes a carbon-oxide gas containing C-14.

15. The method as recited in claim 14, wherein said processing step further comprises:
providing a liquefaction system;
transporting said carbon-oxide gas to said liquefaction system;
converting said carbon-oxide gas to C-14 enriched carbon-oxide; and
processing said C-14 enriched carbon-oxide for disposal.

16. The method as recited in claim 15, wherein said liquefaction system is an amine based CO₂ recovery and liquefaction system.

17. The method as recited in claim 15, wherein said liquefaction system includes a condenser, a vaporizer, a CO converter and a PSA separator, wherein said condenser, said vaporizer, said CO converter and said PSA separator are operatively connected.

18. The method as recited in claim 17, wherein said carbon-oxide gas includes CO containing C-14, and wherein said converting step further comprises:
separating said CO containing C-14 from the remaining carbon-oxide gas in said PSA separator; and
converting said CO containing C-14 to C-14 enriched carbon-oxide.

19. The method as recited in claim 15, wherein the step of processing said C-14 enriched carbon-oxide for disposal comprises converting said C-14 enriched carbon-oxide to a carbon containing compound.

20. The method as recited in claim 19, wherein said carbon containing compound comprises a carbonate, a carbide, or a silicon carbide.

21. The method as recited in claim 1, wherein said first amount of radionuclides includes a gas stream having fine particles, water containing H-3 and HCl containing Cl-36. and wherein said step of removing said first amount of radionuclides from said graphite comprises:
providing a roaster condenser scrubber that is operatively connected to said roaster; and
converting said HCl containing Cl-36 to a salt containing Cl-36.

22. The method as recited in claim 21, further comprising:
condensing said water containing H-3 from said gas stream with said roaster condenser scrubber.

23. The method as recited in claim 22, further comprising:
providing a slurry concentrator filter that is operatively connected to said roaster condenser scrubber;
transporting said condensed water containing H-3 and said Cl-36 salt to said slurry concentrator filter, wherein said water containing H-3 includes undissolved solids; and
filtering said undissolved solids from said condensed water containing H-3.

24. The method as recited in claim 23, further comprising:
providing a boiler that is operatively connected with said roaster condenser scrubber; and
transporting said water containing H-3 and said CI-36 salt to said boiler.

25. The method as recited in claim 21, further comprising:
providing a mineralization unit, wherein said mineralization unit is a wet scrubber; and
transporting said gas stream to said mineralization unit, wherein said gas stream includes CO₂.
reacting said CO₂ with a base.

26. The method as recited in claim 25, further comprising;
reacting said CO₂ with a caustic agent to form a soluble carbonate, wherein said caustic agent comprises NaOH or another basic material; and
discharging said soluble carbonate as a liquid.

27. The method as recited in claim 25, further comprising:
reacting said CO₂ with a caustic agent to form a mineral, wherein said caustic agent comprises lime or another basic material; and
discharging said mineral as a liquid slurry or solid.

28. The method as recited in claim 1, wherein said processing step further comprises:
providing a PSA separator that is operatively connected to said roaster, wherein said first amount of radionuclides includes compounds having an amount of C-14;
passing said compounds through said PSA separator so that said compounds become C-14 enriched; and
providing a mineralization unit that is operatively connected to said PSA separator.

29. The method as recited in claim 28, further comprising:
passing said C-14 enriched compounds through said mineralization unit to form a C-14 containing mineral that is a liquid; and
discharging said liquid.

30. The method as recited in claim 28, further comprising:
providing a solidification unit;
passing said C-14 enriched compounds through said solidification unit to form a C-14 containing solid; and
discharging said C-14 containing solid.

31. The method as recited in claim 29, wherein said liquid includes undissolved solids, and wherein said undissolved are carbonates.

32. The method as recited in claim 1, wherein said processing step further comprises:
providing a CO₂ liquefaction system that is operatively connected to said roaster, wherein said first amount of radionuclides includes CO₂ containing C-14;
discharging said CO₂ containing C-14 as liquid CO₂ through the use of said liquefaction system.

33. The method recited in claim 1, wherein said processing step further comprises:
providing a CO₂ liquefaction system that is operatively connected to said roaster, wherein said first amount of radionuclides includes CO₂ containing C-14;
liquifying said CO₂ containing C-14 in said CO₂ liquefaction system;
discharging said CO₂ containing C-14 as gaseous CO₂ through the use of liquid CO₂.

34. The method as recited in claim 1, further comprising:
reacting said graphite with an additive in said steam reformer to form a liquid; and
discharging said liquid from said steam reformer.

35. The method as recited in claim 34, wherein said liquid is a dissolved solid in a liquid.

36. The method as recited in claim 35, wherein said dissolved solid is a carbonate and wherein said liquid is water.

37. The method as recited in claim 1, wherein said processing step further comprises:
providing a CO₂ liquefaction system that is operatively connected to said steam reformer, wherein said second amount of radionuclides includes an amount of CO₂ having of C-14;
passing said amount of CO₂ through said CO₂ liquefaction system; and
discharging said amount of CO₂ as liquid CO₂.

38. The method as recited in claim 1, further comprising:
providing a moisture adsorber that is operatively connected to said steam reformer, wherein said graphite includes an amount of CO₂ containing C-14;
passing said amount of CO₂ containing C-14 through said moisture adsorber; and
discharging said amount of CO₂ containing C-14 as gas.

39. The method as recited in claim 3, further comprising:
discharging said carbon dioxide from said steam reformer.

40. The method as recited in claim 1, wherein said processing step further comprises:
providing a CO₂ liquefaction system and a CO₂ vaporization system that are operatively connected to said steam reformer, wherein said second amount of radionuclides includes an amount of CO₂ having of C-14;
passing said amount of CO₂ through said CO₂ liquefaction system and said CO₂ vaporization system; and
discharging said amount of CO₂ as gas.

41. The method as recited in claim 1, further comprising:
providing a boiler that is operatively connected to said roaster and said steam reformer, wherein said graphite includes an amount of H-3, and wherein said boiler includes an amount of boiler blowdown;
converting said amount of H-3 to H₂O;
passing said H₂O through said boiler to form steam; and
discharging said boiler blowdown with said H₂O as liquid.

42. The method as recited in claim 1, further comprising:
providing a solidification system that is operatively connected to said roaster and said steam reformer, wherein said graphite includes an amount of H-3;
reacting said amount of H-3 with an oxidizing agent to form H₂O containing H-3:
solidifying said H₂O containing H-3 in said solidification system; and
discharging said solidified H₂O containing H-3.

43. The method as recited in claim 1, wherein said graphite includes an amount of H-3, and wherein said method further comprises:
reacting said amount of H-3 with an oxidizing agent in said steam reformer to form water vapor;
providing a moisture adsorber that is operatively connected to said steam reformer; and
removing said water vapor by said moisture adsorber.

44. The method as recited in claim 43, further comprising:
providing a boiler that is operatively connected to said steam reformer; and
recycling said water vapor to said boiler.

45. The method as recited in claim 1, further comprising:
providing a slurry concentrator filter that is operatively connected to said steam reformer, wherein said graphite includes an amount of non-volatile radionuclides, wherein said step of reacting said graphite with a reforming agent in said steam reformer to form a carbon oxide results in graphite ash; and
concentrating by said slurry concentrator filter said non-volatile radionuclides and said graphite ash.

46. The method as recited in claim 1, further comprising:
providing an additive to said steam reformer, wherein said step of reacting said graphite with a reforming agent in said steam reformer to form a carbon oxide results in graphite ash; and
mineralizing said graphite ash by said additive.

47. The method as recited in claim 46, wherein said mineralizing step comprises converting said graphite ash to a mineral, and wherein said mineral comprises an alkali aluminosilicate, an aluminate, a calcium-based compound, or a phosphate-based compound.

48. The method as recited in claim 1, further comprising:
providing an additive to said steam reformer, wherein said graphite includes an amount of metals; and
converting said metals to water insoluble metal spinels by said additive.

49. The method as recited in claim 48, wherein said metals are heavy metals, wherein said additive is iron, and wherein said insoluble metal spinels are insoluble iron spinels.

50. The method as recited in claim 1, further comprising:
providing an iron containing additive to said steam reformer, wherein said graphite includes an amount of iron;
converting said amount of iron to iron spinels by said iron containing additive.

51. The method as recited in claim 1, further comprising:
providing a slurry concentrator filter that is operatively connected to said steam reformer, wherein said graphite includes an amount of non-volatile radionuclides, and wherein said step of reacting said graphite with a reforming agent in said steam reformer to form a carbon oxide results in graphite ash;
reacting an iron containing additive with said amount of non-volatile radionuclides and said graphite ash to form magnetic iron-based wastes, wherein said slurry concentrator filter includes means to separate said magnetic iron-based wastes and means to concentrate iron spinels, other metal spinels, iron metal oxides, other metal oxides, and iron-based mineral forms.

52. The method as recited in claim 1, wherein said graphite includes an amount of Cl-36, and wherein said method further comprises converting said amount of Cl-36 in said steam reformer and in said roaster to an alkali or an alkaline earth metal chloride for discharge as a water-based liquid with dissolved Cl-36 salts or other water soluble compounds.

53. The method as recited in claim 52, further comprising:
providing an additive to said steam reformer;
converting said alkali and said alkaline earth metal chloride into a water insoluble mineral;
discharging said water insoluble mineral as a solid or slurry.

54. The method as recited in claim 53, wherein said additive comprises aluminum, an aluminum-silicate, or a phosphate compound.

55. The method as recited in claim 1, further comprising:
providing a boiler that is operatively connected to said steam reformer or said roaster, wherein said graphite includes an amount of Cl-36, and wherein said boiler includes an amount of blowdown water; and
converting said amount of Cl-36 in said steam reformer or in said roaster to an alkali or an alkaline earth metal chloride for discharge as a water-based liquid with dissolved Cl-36 salts or other water soluble compounds through the use of said blowdown water from said boiler.

56. The method as recited in claim 1, further comprising:
providing a slurry concentrator filter and a solidification system that are operatively connected to said steam reformer or said roaster, wherein said graphite includes an amount of Cl-36;
converting in said slurry concentrator filter said amount of Cl-36 from said steam reformer or from said roaster to an alkali or an alkaline earth metal chloride for discharge as a water-based liquid with dissolved Cl-36 salts or other water soluble compounds; and
disposing said amount of Cl-36 as a solid carbonate or a solid chlorine-containing mineral through the use of said solidification system.

57. The method as recited in claim 1, further comprising:
providing a mineralization unit that is operatively connected to said steam reformer or said roaster, wherein said graphite includes an amount of Cl-36;
providing an additive to said mineralization unit; and
converting said amount of Cl-36 in said steam reformer or in said roaster to an alkali alumino-silicate or other water insoluble mineral forms for discharge through the use of said mineralization unit.

58. The method as recited in claim 57, wherein said additive comprises clay, phosphate, iron, silica, or aluminum compounds.

59. The method as recited in claim 1, further comprising:
providing a mineralization unit and a solidification system that are operatively connected to said steam reformer or said roaster, wherein said graphite includes an amount of Cl-36;
converting in said steam reformer or said roaster said amount of Cl-36 to solid waste for discharge through the use of said mineralization unit and said solidification system.

60. The method as recited in claim 1, further comprising:
providing a slurry concentrator filter and a solidification system that are operatively connected to said steam reformer or said roaster;
forming in said steam reformer or said roaster metal oxides, metal spinels, and mineral forms, wherein said metal oxides include an amount of insoluble metal oxides, wherein said metal spinels include an amount of insoluble metal spinels, and wherein said mineral forms include an amount of insoluble mineral forms;
concentrating by said slurry concentrator filter said insoluble metal oxides, said insoluble metal spinels, and said insoluble mineral forms; and
transferring said concentrated insoluble metal oxides, insoluble metal spinets, and insoluble mineral forms to said solidification system for disposal as solid waste.

61. The method as recited in claim 1, further comprising:
providing a slurry concentrator filter and a boiler that are operatively connected to said steam reformer or said roaster, wherein said slurry concentrator filter filters water that is used and formed said boiler.

62. The method as recited in claim 1, further comprising:
providing a graphite gasification cooler that is operatively connected to said steam reformer, wherein said heating step and said reacting step result in an outlet gas, wherein said outlet gas includes Cl-36, steam, C-14 carbon-containing gases, H-3 water vapor, and particulate solids;
scrubbing or adsorbing by said graphite gasification cooler said Cl-36;
condensing said steam and H-3 water vapor by said graphite gasification cooler; and
scrubbing and removing said particulate solids as metal oxides, metal spinels, and graphite fines by said graphite gasification cooler.

63. The method as recited in claim 1, further comprising:
providing a roaster gasification condenser, wherein said reacting step results in an outlet gas that contains an amount of Cl-36, steam, C-14 carbon-containing gases, and H-3 water vapor;
cooling said outlet gas by said roaster gasification condenser;
adsorbing or scrubbing said Cl-36 by said roaster gasification condenser; and
condensing said steam and H-3 water vapor by said roaster gasification condenser.

64. The method as recited in claim 1, wherein said roaster is electrically heated.

65. The method as recited in claim 1, further comprising introducing purge gases into said roaster, wherein said purge gases comprise argon, helium, nitrogen, CO₂, CO, oxygen, oxygen containing gases, or steam.

66. The method as recited in claim 65, wherein said purge gases flow countercurrent to said graphite.

67. The method as recited in claim 1, further comprising introducing pressure cycling in said roaster.

68. The method as recited in claim 1, further comprising introducing vacuum cycling in said roaster.

69. The method as recited in claim 68, further comprising introducing pressure cycling in said roaster.

70. The method as recited in claim 1, wherein said roaster is operated at a temperature between about 600°C and about 1200°C.

71. The method as recited in claim 1, wherein said roaster is operated at a temperature between about 800°C and about 1100°C.

72. The method as recited in claim 1, wherein said oxidizing agent comprises oxygen or oxygen containing gas.

73. The method as recited in claim 1, further comprising:
providing a roaster condenser scrubber and a boiler that are operatively connected to said roaster, wherein said graphite includes an amount of H-3;
reacting said amount of H-3 with an oxidizing agent to form H2O containing H-3; and
recycling by said roaster condenser scrubber said H₂O containing H-3 to said boiler to concentrate said amount of H-3.

74. The method as recited in claim 1, further comprising:
providing a roaster condenser scrubber that is operatively connected to said roaster, wherein said graphite includes an amount of Cl-36; and
removing by said roaster condenser scrubber said amount of Cl-36.

75. The method as recited in claim 1, wherein said steam reformer has an operation mode.

76. The method as recited in claim 75, wherein said operation mode is fluidized.

77. The method as recited in claim 75, wherein said operation mode is a fixed bed below a fluidized bed.

78. The method as recited in claim 75, wherein said operation mode is a partially spouted bed with and without a fluidized bed on top of said partially spouted bed.

79. The method as recited in claim 75, wherein said operation mode is a fully spouted bed with and without a fluidized bed on top of said fully spouted bed.

80. The method as recited in claim 75, wherein said operation mode is a spouted bed with fluidizing gas with and without a fluidized bed on top of said spouted bed.

81. The method as recited in claim 1, wherein said steam reformer is operated at a temperature between about 800°C and about 1500°C.

82. The method as recited in claim 1, wherein said steam reformer is operated at a temperature between about 1000°C and about 1300°C.

83. The method as recited in claim 1, further comprising introducing water into said steam reformer to cool contents in said steam reformer.

84. The method as recited in claim 1, further comprising introducing water with an oxygen-containing atomizing gas into said steam reformer to cool contents in said steam reformer.

85. The method as recited in claim 1, wherein said heating step and reacting step result in graphite fines, and wherein said method further comprises recycling to said steam reformer said graphite fines, and substantially gasifying said graphite fines in said steam reformer.

86. The method as recited in claim 1, wherein said heating step and reacting step result in graphite fines, and wherein said method further comprises recycling said graphite fines to said steam reformer in a water-based slurry, and substantially gasifying said graphite fines in said steam reformer.

87. The method as recited in claim 1, wherein said heating step and reacting step result in graphite fines, and wherein said method further comprises recycling said graphite fines to said steam reformer in a water-based slurry and co-injecting oxygen containing gas in said steam reformer, and substantially gasifying said graphite fines.

88. The method as recited in claim 1, wherein said heating step and reacting step result in graphite fines, and wherein said method further comprises recycling said graphite fines to said steam reformer in a water-based slurry, co-injecting oxygen containing gas to substantially gasify said graphite fines in said steam reformer, and adding water simultaneous to said co-injecting step to cool the contents of said steam reformer, wherein said water is atomized by said oxygen-containing gas.

89. The method as recited in claim 1, wherein said heating step and reacting step result in graphite fines, and wherein said method further comprises providing a dry pneumatic transfer system, recycling said graphite fines to said steam reformer with said dry pneumatic transfer system, and substantially gasifying said graphite fines.

90. The method as recited in claim 1, wherein said reforming agent and said oxidizing agent are a fluidizing gas.

91. The method as recited in claim 1, wherein said reforming agent and said oxidizing agent are a water and oxygen containing gas.

92. The method as recited in claim 1, wherein said reforming agent is a fluidizing gas and wherein said oxidizing agent is a water containing gas.

93. The method as recited in claim 1, wherein said reforming agent is a fluidizing gas and wherein said oxidizing agent is a water and oxygen containing gas.

94. The method as recited in claim 1, wherein said reforming agent is a fluidizing gas and wherein said oxidizing agent is an oxygen containing gas.

95. The method as recited in claim 1, wherein said steam reformer includes a bed of graphite, wherein said reacting step results in the formation of hydrogen, and wherein said reacting step further comprises reacting said hydrogen and said carbon oxide with an oxidizing agent to form water and carbon dioxide, wherein said reacting step occurs in the upper portion of said bed.

96. The method as recited in claim 1, wherein said steam reformer includes a bed of graphite, wherein said reacting step results in the formation of hydrogen, and wherein said reacting step further comprises reacting said hydrogen and said carbon oxide with an oxidizing agent to form water and carbon dioxide, wherein said reacting step occurs above said bed.

97. The method as recited in claim 1, further comprising providing means for sizing graphite that is operatively connected to said steam reformer.

98. The method as recited in claim 1, wherein said roaster operates independently of said steam reformer.

99. The method as recited in claim 1, wherein said graphite includes an amount of hydrogen, and wherein said method further comprises reacting said amount of hydrogen with an oxidizing agent to form water in said steam reformer, and cooling said water by injecting additional water into the steam reformer.

100. The method as recited in claim 1, further comprising cooling the contents in said steam reformer by adding water and oxygen-containing atomizing gas.

## Patentansprüche

1. Verfahren zum Graphitabbau und Abfangen von Radionukliden, umfassend:
das Bereitstellen von Radionuklide enthaltendem Graphit;
das Bereitstellen eines Rösters;
das Erwärmen des Graphits in dem Röster;
das Entfernen einer ersten Menge von Radionukliden von dem Graphit;
das Bereitstellen eines Dampfreformers;
das Umsetzen des Graphits mit einem Reformierungsmittel in dem Dampfreformer, um ein Kohlenoxid zu bilden;
das Entfernen einer zweiten Menge von Radionukliden von dem Graphit;
das Verarbeiten der ersten Menge und zweiten Menge von Radionukliden.

2. Verfahren nach Anspruch 1, wobei das Kohlenoxid Kohlenmonoxid ist.

3. Verfahren nach Anspruch 2, weiter umfassend:
das Umsetzen des Kohlenmonoxids mit einem Oxidationsmittel in dem Dampfreformer, um Kohlendioxid zu bilden.

4. Verfahren nach Anspruch 1, weiter umfassend:
das Bereitstellen eines Dimensionierungsmittels, das operativ mit dem Röster verbunden ist, und
das Dimensionieren des Graphits mit dem Dimensionsierungsmittel.

5. Verfahren nach Anspruch 4, wobei das Dimensionierungsmittel ein Zerkleinerer ist, der bemessen ist, die Größe des Graphits auf Stücke zu verringern, die etwa weniger als 20 mm ausmachen, während auch die potentielle Erzeugung von Graphitfeinteilen verringert wird.

6. Verfahren nach Anspruch 4, wobei das Dimensionierungsmittel bei einer geringen Geschwindigkeit betrieben wird, die eine geringe Menge an Feinteilen erzeugt.

7. Verfahren nach Anspruch 6, wobei die geringe Geschwindigkeit etwa weniger als 100 UpM beträgt, und wobei die geringe Menge etwa weniger als 10% beträgt.

8. Verfahren nach Anspruch 6, wobei die geringe Menge etwa weniger als 5% beträgt.

9. Verfahren nach Anspruch 4, wobei das Dimensionierungsmittel ein Inertgaspolster beinhaltet.

10. Verfahren nach Anspruch 9, wobei das Inertgaspolster aus einem oder mehreren der folgenden, einschließlich Argon, Stickstoff und CO₂, hergestellt ist.

11. Verfahren nach Anspruch 4, wobei das Dimensionierungsmittel ein Sperrwasser beinhaltet.

12. Verfahren nach Anspruch 11, weiter umfassend die Schritte des Bereitstellens von Mitteln zum Aufschlämmungsübertrag und des Übertragens des Graphits von einem Reaktorkern in das Dimensionierungsmittel.

13. Verfahren nach Anspruch 4, wobei das Dimensionierungsmittel Hochdruckwasser ist.

14. Verfahren nach Anspruch 1, wobei die erste Menge von Radionukliden ein C-14 enthaltendes Kohlenoxidgas beinhaltet.

15. Verfahren nach Anspruch 14, wobei der Verarbeitungsschritt weiter umfasst:
das Bereitstellen eines Verflüssigungssystems;
das Transportieren des Kohlenoxidgases in das Verflüssigungssystem;
das Umwandeln des Kohlenoxidgases in C-14-angereichertes Kohlenoxid; und
das Verarbeiten des C-14-angereicherten Kohlenoxids zur Beseitigung.

16. Verfahren nach Anspruch 15, wobei das Verflüssigungssystem ein auf Amin basierendes CO₂-Wiedergewinnungs- und Verflüssigungssystem ist.

17. Verfahren nach Anspruch 15, wobei das Verflüssigungssystem einen Kondensator, einen Verdampfer, einen CO-Umwandler und einen PSA-Separator beinhaltet, wobei der Kondensator, der Verdampfer, der CO-Umwandler und der PSA-Separator operativ verbunden sind.

18. Verfahren nach Anspruch 17, wobei das Kohlenoxidgas C-14 enthaltendes CO beinhaltet, und wobei der Umwandlungsschritt weiter umfasst:
das Separieren des C-14 enthaltenden CO von dem verbleibenden Kohlenoxidgas in dem PSA-Separator; und
das Umwandeln des C-14 enthaltenden CO in C-14-angereichertes Kohlenoxid.

19. Verfahren nach Anspruch 15, wobei der Schritt des Verarbeitens des C-14-angereicherten Kohlenoxids zur Beseitigung das Umwandeln des C-14-angereicherten Kohlenoxids in eine Kohlenstoff enthaltende Verbindung umfasst.

20. Verfahren nach Anspruch 19, wobei die Kohlenstoff enthaltende Verbindung ein Carbonat, ein Carbid oder ein Siliciumcarbid umfasst.

21. Verfahren nach Anspruch 1, wobei die erste Menge von Radionukliden einen Gasstrom mit feinen Teilchen, H-3 enthaltendes Wasser und Cl-36 enthaltendes HCl beinhaltet, und wobei der Schritt des Entfernens der ersten Menge von Radionukliden von dem Graphit umfasst:
das Bereitstellen eines Röstkondensierwäschers, der operativ mit dem Röster verbunden ist; und
das Umwandeln des Cl-36 enthaltenden HCl in ein Cl-36 enthaltendes Salz.

22. Verfahren nach Anspruch 21, weiter umfassend:
das Kondensieren des H-3 enthaltenden Wassers von dem Gasstrom mit dem Röstkondensierwäscher.

23. Verfahren nach Anspruch 22, weiter umfassend:
das Bereitstellen eines Aufschlämmungskonzentrationsfilters, der operativ mit dem Röstkondensierwäscher verbunden ist;
das Transportieren des H-3 enthaltenden kondensierten Wassers und des Cl-36-Salzes zu dem Aufschlämmungskonzentrationsfilter, wobei das H-3 enthaltende Wasser unaufgelöste Feststoffe beinhaltet; und
das Filtern der unaufgelösten Feststoffe von dem H-3 enthaltenden kondensierten Wasser.

24. Verfahren nach Anspruch 23, weiter umfassend:
das Bereitstellen eines Kessels, der operativ mit dem Röstkondensierwäscher verbunden ist; und
das Transportieren des H-3 enthaltenden Wassers und des Cl-36-Salzes zu dem Kessel.

25. Verfahren nach Anspruch 21, weiter umfassend:
das Bereitstellen einer Mineralisierungseinheit, wobei die Mineralisierungseinheit ein Naßwäscher ist; und
das Transportieren des Gasstroms zu der Mineralisierungseinheit, wobei der Gasstrom CO₂ beinhaltet;
das Umsetzen des CO₂ mit einer Base.

26. Verfahren nach Anspruch 25, weiter umfassend:
das Umsetzen des CO₂ mit einem kaustischen Mittel, um ein lösliches Carbonat zu bilden, wobei das kaustische Mittel NaOH oder ein anderes basisches Material umfasst; und
das Entnehmen des löslichen Carbonats als eine Flüssigkeit.

27. Verfahren nach Anspruch 25, weiter umfassend:
das Umsetzen des CO₂ mit einem kaustischen Mittel, um ein Mineral zu bilden, wobei das kaustische Material Kalk oder ein anderes basisches Material umfasst; und
das Entnehmen des Minerals als eine flüssige Aufschlämmung oder Feststoff.

28. Verfahren nach Anspruch 1, wobei der Verarbeitungsschritt weiter umfasst:
das Bereitstellen eines PSA-Separators, der operativ mit dem Röster verbunden ist, wobei die erste Menge von Radionukliden Verbindungen mit einer Menge von C-14 beinhaltet;
das Durchführen der Verbindungen durch den PSA-Separator derart, dass die Verbindung C-14-angereichert werden; und
das Bereitstellen einer Mineralisierungseinheit, die operativ mit dem PSA-Separator verbunden ist.

29. Verfahren nach Anspruch 28, weiter umfassend:
das Durchführen der C-14-angereicherten Verbindungen durch die Mineralisierungseinheit, um einen C-14 enthaltendes Mineral, das eine Flüssigkeit ist, zu bilden; und
das Entnehmen der Flüssigkeit.

30. Verfahren nach Anspruch 28, weiter umfassend:
das Bereitstellen einer Verfestigungseinheit;
das Durchführen der C-14-angereicherten Verbindungen durch die Verfestigungseinheit, um einen C-14 enthaltenden Feststoff zu bilden; und
das Entnehmen des C-14 enthaltenden Feststoffs.

31. Verfahren nach Anspruch 29, wobei die Flüssigkeit unaufgelöste Feststoffe beinhaltet, und wobei die unaufgelösten Carbonate sind.

32. Verfahren nach Anspruch 1, wobei der Verarbeitungsschritt weiter umfasst:
das Bereitstellen eines CO₂-Verflüssigungssystems, das operativ mit dem Röster verbunden ist, wobei die erste Menge von Radionukliden C-14 enthaltendes CO₂ beinhaltet;
das Entnehmen des C-14 enthaltenden CO₂ als flüssiges CO₂ durch die Verwendung des Verflüssigungssystems.

33. Verfahren nach Anspruch 1, wobei der Verarbeitungsschritt weiter umfasst:
das Bereitstellen eines CO₂-Verflüssigungssystems, das operativ mit dem Röster verbunden ist, wobei die erste Menge von Radionukliden C-14 enthaltendes CO₂ beinhaltet;
das Verflüssigen des C-14 enthaltenden CO₂ in dem CO₂-Verflüssigungssystem;
das Entnehmen des C-14 enthaltenden CO₂ als gasförmiges CO₂ durch die Verwendung von flüssigem CO₂.

34. Verfahren nach Anspruch 1, weiter umfassend:
das Umsetzen des Graphits mit einem Additiv in dem Dampfreformer, um eine Flüssigkeit zu bilden; und
das Entnehmen der Flüssigkeit aus dem Dampfreformer.

35. Verfahren nach Anspruch 34, wobei die Flüssigkeit ein in einer Flüssigkeit aufgelöster Feststoff ist.

36. Verfahren nach Anspruch 35, wobei der aufgelöste Feststoff ein Carbonat ist, und wobei die Flüssigkeit Wasser ist.

37. Verfahren nach Anspruch 1, wobei der Verarbeitungsschritt weiter umfasst:
das Bereitstellen eines CO₂-Verflüssigungssystems, das operativ mit dem Dampfreformer verbunden ist, wobei die zweite Menge von Radionukliden eine Menge von C-14 aufweisendem CO₂ beinhaltet;
das Durchführen der Menge von CO₂ durch das CO₂-Verflüssigungssystem; und
das Entnehmen der Menge von CO₂ als flüssiges CO₂.

38. Verfahren nach Anspruch 1, weiter umfassend:
das Bereitstellen eines Feuchtigkeitsadsorbers, der operativ mit dem Dampfreformer verbunden ist, wobei das Graphit eine Menge von C-14 enthaltendem CO₂ beinhaltet;
das Durchführen der Menge von C-14 enthaltendem CO₂ durch den Feuchtigkeitsadsorber; und
das Entnehmen der Menge von C-14 enthaltendem CO₂ als Gas.

39. Verfahren nach Anspruch 3, weiter umfassend:
das Entnehmen des Kohlendioxids aus dem Dampfreformer.

40. Verfahren nach Anspruch 1, wobei der Verarbeitungsschritt weiter umfasst:
das Bereitstellen eines CO₂-Verflüssigungssystems und eines CO₂-Verdampfungssystems, die operativ mit dem Dampfreformer verbunden sind, wobei die zweite Menge von Radionukliden eine Menge von C-14 aufweisendem CO₂ beinhaltet;
das Durchführen der Menge von CO₂ durch das CO₂-Verflüssigungssystem und das CO₂-Verdampfungssystem; und
das Entnehmen der Menge von CO₂ als Gas.

41. Verfahren nach Anspruch 1, weiter umfassend:
das Bereitstellen eines Kessels, der operativ mit dem Röster und dem Dampfreformer verbunden ist, wobei das Graphit eine Menge von H-3 beinhaltet, und wobei der Kessel eine Menge von Kessellauge beinhaltet;
das Umwandeln der Menge von H-3 in H₂O;
das Durchführen des H₂O durch den Kessel, um Dampf zu bilden; und
das Entnehmen der Kessellauge mit dem H₂O als Flüssigkeit.

42. Verfahren nach Anspruch 1, weiter umfassend:
das Bereitstellen eines Verfestigungssystems, das operativ mit dem Röster
und dem Dampfreformer verbunden ist, wobei das Graphit eine Menge von H-3 beinhaltet;
das Umsetzen der Menge von H-3 mit einem Oxidationsmittel, um H-3 enthaltendes H₂O zu bilden;
das Verfestigen des H-3 enthaltenden H₂O in dem Verfestigungssystem; und
das Entnehmen des verfestigten H-3 enthaltenden H₂O.

43. Verfahren nach Anspruch 1, wobei das Graphit eine Menge von H-3 beinhaltet, und wobei das Verfahren weiter umfasst:
das Umsetzen der Menge von H-3 mit einem Oxidationsmittel in dem Dampfreformer, um Wasserdampf zu bilden;
das Bereitstellen eines Feuchtigkeitsadsorbers, der operativ mit dem Dampfreformer verbunden ist; und
das Entfernen des Wasserdampfes durch den Feuchtigkeitsadsorber.

44. Verfahren nach Anspruch 43, weiter umfassend:
das Bereitstellen eines Kessels, der operativ mit dem Dampfreformer verbunden ist; und
das Wiedergewinnen des Wasserdampfes in den Kessel.

45. Verfahren nach Anspruch 1, weiter umfassend:
das Bereitstellen eines Aufschlämmungskonzentrationsfilters, der operativ mit dem Dampfreformer verbunden ist, wobei das Graphit eine Menge von nicht-flüchtigen Radionukliden beinhaltet, wobei der Schritt des Umsetzens des Graphits mit einem Reformierungsmittel in dem Dampfreformer, um ein Kohlenoxid zu bilden, Graphitasche ergibt; und
das Konzentrieren der nicht-flüchtigen Radionuklide und der Graphitasche durch den Aufschlämmungskonzentrationsfilter.

46. Verfahren nach Anspruch 1, weiter umfassend:
das Zuführen eines Additivs in den Dampfreformer, wobei der Schritt des Umsetzens des Graphits mit einem Reformierungsmittel in dem Dampfreformer, um ein Kohlenoxid zu bilden, Graphitasche ergibt; und
das Mineralisieren der Graphitasche durch das Additiv.

47. Verfahren nach Anspruch 46, wobei der Mineralisierungsschritt das Umwandeln der Graphitasche in ein Mineral umfasst, und wobei das Mineral ein Alkalialumosilikat, ein Aluminat, eine auf Calcium basierende Verbindung oder eine auf Phosphat basierende Verbindung umfasst.

48. Verfahren nach Anspruch 1, weiter umfassend:
das Zuführen eines Additivs in den Dampfreformer, wobei das Graphit eine Menge von Metallen beinhaltet; und
das Umwandeln der Metalle in wasserunlösliche Metallspinelle durch das Additiv.

49. Verfahren nach Anspruch 48, wobei die Metalle Schwermetalle sind, wobei das Additiv Eisen ist, und wobei die unlöslichen Metallspinelle unlösliche Eisenspinelle sind.

50. Verfahren nach Anspruch 1, weiter umfassend:
das Zuführen eines Eisen enthaltenden Additivs in den Dampfreformer, wobei das Graphit eine Menge von Eisen beinhaltet;
das Umwandeln der Menge von Eisen in Eisenspinelle durch das Eisen enthaltende Additiv.

51. Verfahren nach Anspruch 1, weiter umfassend:
das Bereitstellen eine Aufschlämmungskonzentrationsfilters, der operativ mit dem Dampfreformer verbunden ist, wobei das Graphit eine Menge von nicht-flüchtigen Radionukliden beinhaltet, und wobei der Schritt des Umsetzens des Graphits mit dem Reformierungsmittel in dem Dampfreformer, um ein Kohlenoxid zu bilden, Graphitasche ergibt;
das Umsetzen eines Eisen enthaltenden Additivs mit der Menge von nicht-flüchtigen Radionukliden und der Graphitasche, um magnetische, auf Eisen basierende Abfälle zu bilden, wobei der Aufschlämmungskonzentrationsfilter Mittel, die magnetischen, auf Eisen basierenden Abfälle abzutrennen, und Mittel, um Eisenspinelle, andere Metallspinelle, Eisenmetalloxide, andere Metalloxide und auf Eisen basierende mineralische Formen aufzukonzentrieren, beinhaltet.

52. Verfahren nach Anspruch 1, wobei das Graphit eine Menge von Cl-36 beinhaltet, und wobei das Verfahren weiter das Umwandeln der Menge von Cl-36 in dem Dampfreformer und in dem Röster in ein Alkali- oder ein Erdalkalimetallchlorid zur Entnahme als eine auf Wasser basierende Flüssigkeit mit aufgelösten Cl-36-Salzen oder andere wasserlösliche Verbindungen umfasst.

53. Verfahren nach Anspruch 52, weiter umfassend:
das Zuführen eines Additivs in den Dampfreformer;
das Umwandeln des Alkali- und des Erdalkalimetallchlorids in ein wasserunlösliches Mineral;
das Entnehmen des wasserunlöslichen Minerals als ein Feststoff oder Aufschlämmung.

54. Verfahren nach Anspruch 53, wobei das Additiv Aluminium, ein Alumosilikat oder eine Phosphatverbindung umfasst.

55. Verfahren nach Anspruch 1, weiter umfassend:
das Bereitstellen eines Kessels, der operativ mit dem Dampfreformer oder dem Röster verbunden ist, wobei das Graphit eine Menge von Cl-36 beinhaltet, und wobei der Kessel eine Menge von Kesselwasser beinhaltet; und
das Umwandeln der Menge von Cl-36 in dem Dampfreformer oder in dem Röster in ein Alkali- oder ein Erdalkalimetallchlorid zur Entnahme als eine auf Wasser basierende Flüssigkeit mit aufgelösten Cl-36-Salzen oder anderen wasserlöslichen Verbindungen durch die Verwendung des Kesselwassers von dem Kessel.

56. Verfahren nach Anspruch 1, weiter umfassend:
das Bereitstellen eines Aufschlämmungskonzentrationsfilters und eines Verfestigungssystems, die operativ mit dem Dampfreformer oder dem Röster verbunden sind, wobei das Graphit eine Menge von Cl-36 beinhaltet;
das Umwandeln der Menge von Cl-36 von dem Dampfreformer oder von dem Röster in ein Alkali- oder ein Erdalkalimetallchlorid zur Entnahme als eine auf Wasser basierende Flüssigkeit mit aufgelösten Cl-36-Salzen oder anderen wasserlöslichen Verbindungen; und
das Beseitigen der Menge von Cl-36 als ein festes Carbonat oder ein festes Chlor-enthaltendes Mineral durch die Verwendung des Verfestigungssystems.

57. Verfahren nach Anspruch 1, weiter umfassend:
das Bereitstellen einer Mineralisierungseinheit, die operativ mit dem Dampfreformer oder dem Röster verbunden ist, wobei das Graphit eine Menge von Cl-36 beinhaltet;
das Zuführen eines Additivs in die Mineralisierungseinheit; und
das Umwandeln der Menge von Cl-36 in dem Dampfreformer oder in dem Röster in ein Alkalialumosilikat oder andere wasserunlösliche Mineralformen zur Entnahme durch die Verwendung der Mineralisierungseinheit.

58. Verfahren nach Anspruch 57, wobei das Additiv Ton, Phosphat, Eisen, Siliciumdioxid oder Aluminiumverbindungen umfasst.

59. Verfahren nach Anspruch 1, weiter umfassend:
das Bereitstellen einer Mineralisierungseinheit und eines Verfestigungssystems, die operativ mit dem Dampfreformer oder dem Röster verbunden sind, wobei das Graphit eine Menge von Cl-36 beinhaltet;
das Umwandeln der Menge von Cl-36 in dem Dampfreformer oder dem Röster in festen Abfall zur Entnahme durch die Verwendung der Mineralisierungseinheit und des Verfestigungssystems.

60. Verfahren nach Anspruch 1, weiter umfassend:
das Bereitstellen eines Aufschlämmungskonzentrationsfilters und eines Verfestigungssystems, die operativ mit dem Dampfreformer oder dem Röster verbunden sind;
das Bilden von Metalloxiden, Metallspinellen und Mineralformen in dem Dampfreformer oder dem Röster, wobei die Metalloxide eine Menge von unlöslichen Metalloxiden beinhalten, wobei die Metallspinelle eine Menge von unlöslichen Metallspinellen beinhalten, und wobei die Mineralformen eine Menge von unlöslichen Mineralformen beinhalten;
das Konzentrieren der unlöslichen Metalloxide, der unlöslichen Metallspinelle und der unlöslichen Mineralformen durch den Aufschlämmungskonzentrationsfilter; und
das Überführen der konzentrierten unlöslichen Metalloxide, unlöslichen Metallspinelle und unlöslichen Mineralformen in das Verfestigungssystem zur Beseitigung als fester Abfall.

61. Verfahren nach Anspruch 1, weiter umfassend:
das Bereitstellen eines Aufschlämmungskonzentrationsfilters und eines Kessels, die operativ mit dem Dampfreformer oder dem Röster verbunden sind, wobei der Aufschlämmungskonzentrationsfilter Wasser filtert, das in dem Kessel verwendet und gebildet wird.

62. Verfahren nach Anspruch 1, weiter umfassend:
das Bereitstellen eines Graphitvergasungskühlers, der operativ mit dem Dampfreformer verbunden ist, wobei der Erwärmungsschritt und der Umsetzungsschritt ein Auslaßgas ergeben, wobei das Auslaßgas Cl-36, Dampf, C-14-Kohlenstoff enthaltende Gase, H-3-Wasserdampf und partikuläre Feststoffe beinhaltet;
das Auswaschen oder Adsorbieren des Cl-36 durch den Graphitvergasungskühler;
das Kondensieren des Dampfes und des H-3-Wasserdampfes durch den Graphitvergasungskühler; und
das Waschen und Entfernen der partikulären Feststoffe als Metalloxide, Metalspinelle und Graphitfeinteile durch den Graphitvergasungskühler.

63. Verfahren nach Anspruch 1, weiter umfassend:
das Bereitstellen eines Röstervergasungskondensators, wobei der Umsetzungsschritt ein Auslaßgas ergibt, das eine Menge von Cl-36, Dampf, C-14-Kohlenstoff enthaltende Gase und H-3-Wasserdampf enthält;
das Kühlen des Auslaßgases durch den Röstervergasungskondensator;
das Adsorbieren oder Auswaschen des Cl-36 durch den Röstervergasungskondensator; und
das Kondensieren des Dampfes und des H-3-Wasserdampfes durch den Röstervergasungskondensator.

64. Verfahren nach Anspruch 1, wobei der Röster elektrisch erwärmt wird.

65. Verfahren nach Anspruch 1, weiter umfassend das Einführen von Spülgasen in den Röster, wobei die Spülgase Argon, Helium, Stickstoff, CO₂, CO, Sauerstoff, Sauerstoff enthaltende Gase oder Dampf umfassen.

66. Verfahren nach Anspruch 65, wobei die Spülgase entgegengesetzt zu dem Graphit fließen.

67. Verfahren nach Anspruch 1, weiter umfassend das Einführen von Drucksteuerung in dem Röster.

68. Verfahren nach Anspruch 1, weiter umfassend das Einführen von Vakuumsteuerung in dem Röster.

69. Verfahren nach Anspruch 68, weiter umfassend das Einführen von Drucksteuerung in dem Röster.

70. Verfahren nach Anspruch 1, wobei der Röster bei einer Temperatur zwischen etwa 600°C und etwa 1200°C betrieben wird.

71. Verfahren nach Anspruch 1, wobei der Röster bei einer Temperatur zwischen etwa 800°C und etwa 1100°C betrieben wird.

72. Verfahren nach Anspruch 1, wobei das Oxidationsmittel Sauerstoff oder Sauerstoff enthaltendes Gas umfasst.

73. Verfahren nach Anspruch 1, weiter umfassend:
das Bereitstellen eines Rösterkondensationswäschers und eines Kessels, die operativ mit dem Röster verbunden sind, wobei das Graphit eine Menge von H-3 beinhaltet;
das Umsetzen der Menge von H-3 mit einem Oxidationsmittel, um H-3 enthaltendes H₂O zu bilden; und
das Wiedergewinnen des H-3 enthaltenden H₂O durch den Rösterkondensationswäscher in den Kessel, um die Menge von H-3 zu konzentrieren.

74. Verfahren nach Anspruch 1, weiter umfassend:
das Bereitstellen eines Rösterkondensationswäschers, der operativ mit dem Röster verbunden ist, wobei das Graphit eine Menge von Cl-36 beinhaltet; und
das Entfernen der Menge von Cl-36 durch den Rösterkondensationswäscher.

75. Verfahren nach Anspruch 1, wobei der Dampfreformer eine Betriebsart aufweist.

76. Verfahren nach Anspruch 75, wobei die Betriebsart Fließbett ist.

77. Verfahren nach Anspruch 75, wobei die Betriebsart ein Festbett unter einem Fließbett ist.

78. Verfahren nach Anspruch 75, wobei die Betriebsart ein teilweises Sprudelbett mit oder ohne einem Fließbett auf dem teilweisen Sprudelbett ist.

79. Verfahren nach Anspruch 75, wobei die Betriebsart ein vollständiges Sprudelbett mit oder ohne einem Fließbett auf dem vollständigen Sprudelbett ist.

80. Verfahren nach Anspruch 75, wobei die Betriebsart ein Sprudelbett mit Wirbelgas mit oder ohne einem Fließbett auf dem Sprudelbett ist.

81. Verfahren nach Anspruch 1, wobei der Dampfreformer bei einer Temperatur zwischen etwa 800°C und etwa 1500°C betrieben wird.

82. Verfahren nach Anspruch 1, wobei der Dampfreformer bei einer Temperatur zwischen etwa 1000°C und etwa 1300°C betrieben wird.

83. Verfahren nach Anspruch 1, weiter umfassend das Einführen von Wasser in den Dampfreformer, um Inhalte in dem Dampfreformer zu kühlen.

84. Verfahren nach Anspruch 1, weiter umfassend das Einführen von Wasser mit einem Sauerstoff-enthaltenden Zerstäubergas in den Dampfreformer, um Inhalte in dem Dampfreformer zu kühlen.

85. Verfahren nach Anspruch 1, wobei der Erwärmungsschritt und der Umsetzungsschritt Graphitfeinteile ergeben, und wobei das Verfahren weiter das Wiedergewinnen der Graphitfeinteile in den Dampfreformer und das im Wesentlichen Vergasen der Graphitfeinteile in dem Dampfreformer umfasst.

86. Verfahren nach Anspruch 1, wobei der Erwärmungsschritt und der Umsetzungsschritt Graphitfeinteile ergeben, und wobei das Verfahren weiter das Wiedergewinnen der Graphitfeinteile in den Dampfreformer in einer auf Wasser basierenden Aufschlämmung und das im Wesentlichen Vergasen der Graphitfeinteile in dem Dampfreformer umfasst.

87. Verfahren nach Anspruch 1, wobei der Erwärmungsschritt und der Umsetzungsschritt Graphitfeinteile ergeben, und wobei das Verfahren weiter das Wiedergewinnen der Graphitfeinteile in den Dampfreformer in einer auf Wasser basierenden Aufschlämmung und das Co-injizieren von Sauerstoff enthaltendem Gas in den Dampfreformer und das im Wesentlichen Vergasen der Graphitfeinteile umfasst.

88. Verfahren nach Anspruch 1, wobei der Erwärmungsschritt und der Umsetzungsschritt Graphitfeinteile ergeben, und wobei das Verfahren weiter das Wiedergewinnen der Graphitfeinteile in den Dampfreformer in einer auf Wasser basierenden Aufschlämmung, das Co-injizieren von Sauerstoff enthaltendem Gas, um die Graphitfeinteile in dem Dampfreformer im Wesentlichen zu vergasen, und das Zugeben von Wasser gleichzeitig mit dem Coinjektionsschritt, um die Inhalte des Dampfreformer zu kühlen, umfasst, wobei das Wasser durch das Sauerstoff enthaltende Gas zerstäubt wird.

89. Verfahren nach Anspruch 1, wobei der Erwärmungsschritt und der Umsetzungsschritt Graphitfeinteile ergeben, und wobei das Verfahren weiter das Bereitstellen eines trockenen pneumatischen Übertragungssystems, das Wiedergewinnen der Graphitfeinteile in den Dampfreformer mit dem trockenen pneumatischen Übertragungssystem und das im Wesentlichen Vergasen der Graphitfeinteile umfasst.

90. Verfahren nach Anspruch 1, wobei das Reformierungsmittel und das Oxidationsmittel ein Wirbelgas sind.

91. Verfahren nach Anspruch 1, wobei das Reformierungsmittel und das Oxidationsmittel ein Wasser und Sauerstoff enthaltendes Gas sind.

92. Verfahren nach Anspruch 1, wobei das Reformierungsmittel ein Wirbelgas ist und wobei das Oxidationsmittel ein Wasser enthaltendes Gas ist.

93. Verfahren nach Anspruch 1, wobei das Reformierungsmittel ein Wirbelgas ist und wobei das Oxidationsmittel ein Wasser und Sauerstoff enthaltendes Gas ist.

94. Verfahren nach Anspruch 1, wobei das Reformierungsmittel ein Wirbelgas ist und das Oxidationsmittel ein Sauerstoff enthaltendes Gas ist.

95. Verfahren nach Anspruch 1, wobei der Dampfreformer ein Graphitbett beinhaltet, wobei der Umsetzungsschritt die Bildung von Wasserstoff ergibt, und wobei der Umsetzungsschritt weiter das Umsetzen des Wasserstoffs und des Kohlenoxids mit einem Oxidationsmittel umfasst, um Wasser und Kohlendioxid zu bilden, wobei der Umsetzungsschritt in dem oberen Bereich des Betts auftritt.

96. Verfahren nach Anspruch 1, wobei der Dampfreformer ein Graphitbett beinhaltet, wobei der Umsetzungsschritt die Bildung von Wasserstoff ergibt, und wobei der Umsetzungsschritt weiter das Umsetzen des Wasserstoffs und des Kohlenoxids mit einem Oxidationsmittel umfasst, um Wasser und Kohlendioxid zu bilden, wobei der Umsetzungsschritt über dem Bett auftritt.

97. Verfahren nach Anspruch 1, weiter umfassend das Bereitstellen eines Mittels zum Dimensionieren von Graphit, das operativ mit dem Dampfreformer verbunden ist.

98. Verfahren nach Anspruch 1, wobei der Röster unabhängig von dem Dampfreformer arbeitet.

99. Verfahren nach Anspruch 1, wobei das Graphit eine Menge von Wasserstoff beinhaltet, und wobei das Verfahren weiter das Umsetzen der Menge von Wasserstoff mit einem Oxidationsmittel, um Wasser in dem Dampfreformer zu bilden, und das Kühlen des Wasser durch das Injizieren von zusätzlichem Wasser in den Dampfreformer umfasst..

100. Verfahren nach Anspruch 1, weiter umfassend das Kühlen der Inhalte in dem Dampfreformer durch das Zugeben von Wasser und Sauerstoff enthaltendem Zerstäubergas.

## Revendications

1. Procédé de destruction du graphite et de capture de radionucléides, comprenant les étapes consistant à :
fournir du graphite contenant des radionucléides ;
fournir un four de grillage ;
chauffer ledit graphite dans ledit four de grillage ;
retirer une première quantité de radionucléides dudit graphite ;
fournir un reformeur à vapeur ;
faire réagir ledit graphite avec un agent de reformage dans ledit reformeur à vapeur pour former un oxyde de carbone ;
retirer une seconde quantité de radionucléides dudit graphite ;
traiter ladite première quantité et ladite seconde quantité de radionucléides.

2. Procédé selon la revendication 1, dans lequel ledit oxyde de carbone est du monoxyde de carbone.

3. Procédé selon la revendication 2, comprenant en outre l'étape consistant à :
faire réagir ledit monoxyde de carbone avec un agent oxydant dans ledit reformeur à vapeur pour former du dioxyde de carbone.

4. Procédé selon la revendication 1, comprenant en outre l'étape consistant à :
fournir un moyen de calibrage qui est raccordé en exploitation audit four de grillage ; et
calibrer ledit graphite avec ledit moyen de calibrage.

5. Procédé selon la revendication 4, dans lequel ledit moyen de calibrage est un concasseur dimensionné pour réduire la taille dudit graphite en morceaux d'environ moins de 20 mm, tout en réduisant également la production potentielle de fines de graphite.

6. Procédé selon la revendication 4, dans lequel ledit moyen de calibrage est exploité à une faible vitesse qui génère une faible quantité de fines.

7. Procédé selon la revendication 6, dans lequel ladite faible vitesse est environ inférieure à 100 tpm, et dans lequel ladite faible quantité est environ inférieure à 10 %.

8. Procédé selon la revendication 6, dans lequel ladite faible quantité est environ inférieure à 5 %.

9. Procédé selon la revendication 4, dans lequel ledit moyen de calibrage comprend une couverture gazeuse inerte.

10. Procédé selon la revendication 9, dans lequel ladite couverture gazeuse inerte se compose d'un ou plusieurs des gaz suivants, notamment l'argon, l'azote et le CO₂.

11. Procédé selon la revendication 4, dans lequel ledit moyen de calibrage comprend un joint d'eau.

12. Procédé selon la revendication 11, comprenant en outre les étapes consistant à fournir des moyens pour le transfert de la boue et à transférer ledit graphite du coeur d'un réacteur vers ledit moyen de calibrage.

13. Procédé selon la revendication 4, dans lequel ledit moyen de calibrage est de l'eau sous haute pression.

14. Procédé selon la revendication 1, dans lequel ladite première quantité de radionucléides comprend du gaz oxyde de carbone contenant du C-14.

15. Procédé selon la revendication 14, dans lequel ladite étape de traitement comprend en outre :
fournir un système de liquéfaction ;
transporter ledit gaz oxyde de carbone vers ledit système de liquéfaction ;
convertir ledit gaz oxyde de carbone en oxyde de carbone enrichi en C-14 ; et
traiter ledit oxyde de carbone enrichi en C-14 pour son élimination.

16. Procédé selon la revendication 15, dans lequel ledit système de liquéfaction est un système de récupération de CO₂ et de liquéfaction à base d'amine.

17. Procédé selon la revendication 15, dans lequel ledit système de liquéfaction comprend un condenseur, un évaporateur, un convertisseur de CO et un séparateur par adsorption modulée en pression (PSA), ledit condenseur, ledit évaporateur, ledit convertisseur de CO et ledit séparateur PSA étant raccordés en exploitation.

18. Procédé selon la revendication 17, dans lequel ledit gaz oxyde de carbone comprend CO qui contient du C-14, et dans lequel ladite étape de conversion comprend en outre :
la séparation dudit CO contenant du C-14 du gaz oxyde de carbone restant dans ledit séparateur PSA ; et
la conversion dudit CO contenant du C-14 en oxyde de carbone enrichi en C-14.

19. Procédé selon la revendication 15, dans lequel l'étape de traitement dudit oxyde de carbone enrichi en C-14 destiné à être éliminé comprend la conversion dudit oxyde de carbone enrichi en C-14 en un composé contenant du carbone.

20. Procédé selon la revendication 19, dans lequel ledit composé contenant du carbone comprend un carbonate, un carbure ou un carbure de silicium.

21. Procédé selon la revendication 1, dans lequel ladite première quantité de radionucléides comprend un courant gazeux présentant des particules fines, de l'eau contenant H-3 et HCl contenant du C1-36, et dans lequel ladite étape de retrait de ladite première quantité de radionucléides dudit graphite comprend :
la fourniture d'un four de grillage/condenseur/laveur raccordé en exploitation audit four de grillage ; et
la conversion dudit HCl contenant du Cl-36 en un sel contenant du Cl-36.

22. Procédé selon la revendication 21, comprenant en outre l'étape consistant à :
condenser ladite eau contenant H-3 dudit courant gazeux avec ledit four de grillage/condenseur/laveur.

23. Procédé selon la revendication 22, comprenant en outre les étapes consistant à :
fournir un dit filtre concentrateur de boue qui est raccordé en exploitation audit four de grillage/condenseur/laveur ;
transporter ladite eau condensée contenant H-3 et ledit sel contenant du Cl-36 vers ledit filtre concentrateur de boue, ladite eau contenant H-3 comprenant des solides non dissous ;
filtrer lesdits solides non dissous de ladite eau condensée contenant H-3.

24. Procédé selon la revendication 23, comprenant en outre les étapes consistant à :
fournir une chaudière qui est raccordée en exploitation audit four de grillage/condenseur/laveur ; et
transporter ladite eau contenant H-3 et ledit sel contenant Du Cl-36 vers ladite chaudière.

25. Procédé selon la revendication 21, comprenant en outre les étapes consistant à :
fournir une unité de minéralisation dans laquelle ladite unité de minéralisation est un laveur par voie humide ; et
transporter ledit courant gazeux vers ladite unité de minéralisation, ledit courant gazeux comprenant du CO₂ ;
faire réagir ledit CO₂ avec une base.

26. Procédé selon la revendication 25, comprenant en outre les étapes consistant à :
faire réagir ledit CO₂ avec un agent caustique pour former un carbonate soluble, ledit agent caustique comprenant NaOH ou un autre matériau basique ; et
évacuer ledit carbonate soluble sous la forme d'un liquide.

27. Procédé selon la revendication 25, comprenant en outre les étapes consistant à :
faire réagir ledit CO₂ avec un agent caustique pour former un minéral, où ledit agent caustique comprend de la chaux ou un autre matériau basique ; et
évacuer le minéral sous la forme d'une boue liquide ou d'un solide.

28. Procédé selon la revendication 1, dans lequel ladite étape de traitement comprend en outre :
la fourniture d'un séparateur PSA qui est raccordé en exploitation audit four de grillage, ladite première quantité de radionucléides comprenant des composés qui contiennent une certaine quantité de C-14 ;
le passage desdits composés par ledit séparateur PSA de façon telle que lesdits composés deviennent enrichis en C-14 ; et
la fourniture d'une unité de minéralisation qui est raccordée en exploitation audit séparateur PSA.

29. Procédé selon la revendication 28, comprenant en outre les étapes consistant à :
passer lesdits composés enrichis en C-14 par ladite unité de minéralisation pour former un minéral contenant du C-14 qui est un liquide ; et
évacuer ledit liquide.

30. Procédé selon la revendication 28, comprenant en outre les étapes consistant à :
fournir une unité de solidification ;
passer lesdits composés enrichis en C-14 par ladite unité de solidification pour former un solide contenant du C-14 ; et
évacuer ledit solide contenant du C-14.

31. Procédé selon la revendication 29, dans lequel ledit liquide comprend des solides non dissous, et dans lequel lesdits solides non dissous sont des carbonates.

32. Procédé selon la revendication 1, dans lequel ladite étape de traitement comprend en outre :
la fourniture d'un système de liquéfaction de CO₂ raccordé en exploitation audit four de grillage, ladite première quantité de radionucléides comprenant du CO₂ qui contient du C-14 ;
l'évacuation dudit CO₂ contenant du C-14 sous la forme de CO₂ liquide via l'utilisation dudit système de liquéfaction.

33. Procédé selon la revendication 1, dans lequel ladite étape de traitement comprend en outre :
la fourniture d'un système de liquéfaction de CO₂ qui est raccordé en exploitation audit four de grillage, ladite première quantité de radionucléides comprenant du CO₂ qui contient du C-14 ;
la liquéfaction dudit CO₂ contenant du C-14 dans ledit système de liquéfaction de CO₂ ;
l'évacuation dudit CO₂ contenant du C-14 sous la forme de CO₂ gazeux via l'utilisation de CO₂ liquide.

34. Procédé selon la revendication 1, comprenant en outre les étapes consistant à :
faire réagir ledit graphite avec un additif dans ledit reformeur à vapeur pour former un liquide ; et
évacuer ledit liquide dudit reformeur à vapeur.

35. Procédé selon la revendication 34, dans lequel ledit liquide est un solide dissous dans un liquide.

36. Procédé selon la revendication 35, dans lequel ledit solide dissous est un carbonate et dans lequel ledit liquide est de l'eau.

37. Procédé selon la revendication 1, dans lequel ladite étape de traitement comprend en outre :
la fourniture d'un système de liquéfaction de CO₂ qui est raccordé en exploitation audit reformeur à vapeur, ladite seconde quantité de radionucléides comprenant une quantité de CO₂ qui contient du C-14 ;
le passage de ladite quantité de CO₂ par ledit système de liquéfaction de CO₂ ; et
l'évacuation de ladite quantité de CO₂ sous la forme de CO₂ liquide.

38. Procédé selon la revendication 1, comprenant en outre les étapes consistant à :
fournir un adsorbeur d'humidité qui est raccordé en exploitation audit reformeur à vapeur, dans lequel ledit graphite comprend une quantité de CO₂ qui contient du C-14 ;
passer ladite quantité de CO₂ contenant du C-14 par ledit adsorbeur d'humidité ; et
évacuer ladite quantité de CO₂ contenant du C-14 sous la forme d'un gaz.

39. Procédé selon la revendication 3, comprenant en outre l'étape consistant à :
évacuer ledit dioxyde de carbone dudit reformeur à vapeur.

40. Procédé selon la revendication 1, dans lequel ladite étape de traitement comprend :
la fourniture d'un système de liquéfaction de CO₂ et d'un système de vaporisation de CO₂ qui sont raccordés en exploitation audit reformeur à vapeur, ladite seconde quantité de radionucléides comprenant une quantité de CO₂ qui contient du C-14 ;
le passage de ladite quantité de CO₂ par ledit système de liquéfaction de CO₂ et ledit système de vaporisation de CO₂ ; et
l'évacuation de ladite quantité de CO₂ sous la forme de gaz.

41. Procédé selon la revendication 1, comprenant en outre les étapes consistant à :
fournir une chaudière qui est raccordée en exploitation audit four de grillage et audit reformeur à vapeur, ledit graphite comprenant une quantité de H-3 et ladite chaudière comprenant une quantité de purges de chaudière ;
convertir ladite quantité de H-3 en H₂O ;
passer ledit H₂O par ladite chaudière pour former de la vapeur ; et
évacuer lesdites purges de chaudière avec ledit H₂O sous la forme de liquide.

42. Procédé selon la revendication 1, comprenant en outre les étapes consistant à :
fournir un système de solidification qui est raccordé en exploitation audit four de grillage et audit reformeur à vapeur, ledit graphite comprenant une quantité de H-3 ;
faire réagir ladite quantité de H-3 avec un agent oxydant pour former H₂O contenant H-3 ;
solidifier ledit H₂O contenant H-3 dans ledit système de solidification ; et
évacuer ledit H₂O solidifié contenant H-3.

43. Procédé selon la revendication 1, dans lequel ledit graphite contient une quantité de H-3 et dans lequel ledit procédé comprend en outre les étapes consistant à :
faire réagir ledit H-3 avec un agent oxydant dans ledit reformeur à vapeur pour former de la vapeur d' eau ;
fournir un adsorbeur d'humidité qui est raccordé en exploitation audit reformeur à vapeur ; et
éliminer ladite vapeur d'eau par ledit adsorbeur d'humidité.

44. Procédé selon la revendication 43, comprenant en outre les étapes consistant à :
fournir une chaudière qui est raccordée en exploitation audit reformeur à vapeur ; et
recycler ladite vapeur d'eau vers ladite chaudière.

45. Procédé selon la revendication 1, comprenant en outre les étapes consistant à :
fournir un filtre concentrateur de boue qui est connecté en exploitation audit reformeur à vapeur, ledit graphite comprenant une quantité de radionucléides non volatils, ladite étape de réaction dudit graphite avec un agent de reformage dans ledit reformeur à vapeur pour former un oxyde de carbone donnant de la cendre de graphite ; et
concentrer par ledit filtre concentrateur de boue lesdits radionucléides non volatiles et ladite cendre de graphite.

46. Procédé selon la revendication 1, comprenant en outre les étapes consistant à :
fournir un additif dans ledit reformeur à vapeur, ladite étape de réaction dudit graphite avec un agent de reformage dans ledit reformeur à vapeur pour former un oxyde de carbone donnant de la cendre de graphite ; et
minéraliser ladite cendre de graphite par ledit additif.

47. Procédé selon la revendication 46, dans lequel ladite étape de minéralisation comprend la conversion de ladite cendre de graphite en un minéral, et dans lequel ledit minéral comprend un aluminosilicate alcalin, un aluminate, un composé à base de calcium ou un composé à base de phosphate.

48. Procédé selon la revendication 1, comprenant en outre les étapes consistant à :
fournir un additif dans ledit reformeur à vapeur, ledit graphite comprenant une quantité de métaux ; et
convertir lesdits métaux en spinelles métalliques insolubles par ledit additif.

49. Procédé selon la revendication 48, dans lequel lesdits métaux sont des métaux lourds, dans lequel ledit additif est du fer, et dans lequel lesdits spinelles métalliques insolubles sont des spinelles de fer insolubles.

50. Procédé selon la revendication 1, comprenant en outre les étapes consistant à :
fournir un additif contenant du fer dans ledit reformeur à vapeur, ledit graphite comprenant une quantité de fer ;
convertir ladite quantité de fer en spinelles de fer par ledit additif contenant du fer.

51. Procédé selon la revendication 1, comprenant en outre les étapes consistant à :
fournir un filtre concentrateur de boue qui est raccordé en exploitation audit reformeur à vapeur, ledit graphite comprenant une quantité de radionucléides non volatils, et ladite étape de réaction dudit graphite avec un agent de reformage dans ledit reformeur à vapeur pour former un oxyde de carbone donnant de la cendre de graphite ;
faire réagir ledit additif contenant du fer avec ladite quantité de radionucléides non volatils et ladite centre de graphite pour former des déchets magnétiques à base de fer, ledit filtre concentrateur de boue comprenant un moyen permettant de séparer lesdits déchets magnétiques à base de fer et un moyen permettant de concentrer les spinelles de fer, les autres spinelles métalliques, les oxydes métalliques de fer et d'autres oxydes métalliques, et les formes minérales à base de fer.

52. Procédé selon la revendication 1, dans lequel ledit graphite comprend une quantité de Cl-36 et dans lequel ledit procédé comprend en outre l'étape consistant à convertir ladite quantité de Cl-36 dans ledit reformeur à vapeur et dans ledit four de grillage en un chlorure de métal alcalin ou alcalino-terreux pour être évacué en tant que liquide à base d'eau avec des sels de C1-36 dissous ou d'autres composés solubles dans l'eau.

53. Procédé selon la revendication 52, comprenant en outre les étapes consistant à :
fournir un additif dans ledit reformeur à vapeur ;
convertir ledit chlorure de métal alcalin ou alcalino-terreux en un minéral insoluble dans l'eau ;
évacuer ledit minéral insoluble dans l'eau sous la forme d'un solide ou d'une boue.

54. Procédé selon la revendication 53, dans lequel ledit additif comprend de l'aluminium, un silicate d'aluminium ou un composé de phosphate.

55. Procédé selon la revendication 1, comprenant en outre les étapes consistant à :
fournir une chaudière qui est raccordée en exploitation audit reformeur à vapeur ou audit four de grillage, ledit graphite comprenant une quantité de Cl-36 et ladite chaudière comprenant une quantité d'eau de purge ; et
convertir ladite quantité de Cl-36 dans ledit reformeur à vapeur ou dans ledit four de grillage en un chlorure de métal alcalin ou alcalino-terreux pour l'évacuer sous la forme d'un liquide à base d'eau avec des sels contenant Du Cl-36 dissous ou d'autres composés solubles dans l'eau via l'utilisation de ladite eau de purge de ladite chaudière.

56. Procédé selon la revendication 1, comprenant en outre les étapes consistant à :
fournir un filtre concentrateur de boue et un système de solidification qui sont raccordés en exploitation audit reformeur à vapeur ou audit four de grillage, ledit graphite comprenant une quantité de Cl-36 ;
convertir dans ledit filtre concentrateur de boue ladite quantité de Cl-36 depuis ledit reformeur à vapeur ou depuis ledit four de grillage en un chlorure de métal alcalin ou alcalino-terreux pour l'évacuer sous la forme d'un liquide à base d'eau avec des sels contenant Du C1-36 dissous ou d'autres composés solubles dans l' eau ; et
évacuer ladite quantité de C1-36 sous la forme d'un carbonate solide ou d'un minéral solide contenant du chlore via l'utilisation dudit système de solidification.

57. Procédé selon la revendication 1, comprenant en outre les étapes consistant à :
fournir une unité de minéralisation qui est raccordée en exploitation audit reformeur à vapeur ou audit four de grillage, ledit graphite comprenant une quantité de Cl-36 ;
fournir un additif dans l'unité de minéralisation ; et
convertir ladite quantité de Cl-36 dans ledit reformeur à vapeur ou dans ledit four de grillage en un aluminosilicate alcalin ou d'autres formes de minéraux insolubles dans l'eau pour l'évacuer via l'utilisation de ladite unité de minéralisation.

58. Procédé selon la revendication 57, dans lequel ledit additif comprend de l'argile, du phosphate, du fer, de la silice ou des composés d'aluminium.

59. Procédé selon la revendication 1, comprenant en outre les étapes consistant à :
fournir une unité de minéralisation et un système de solidification qui sont raccordés en exploitation audit reformeur à vapeur ou audit four de grillage, ledit graphite comprenant une quantité de Cl-36 ;
convertir dans ledit reformeur à vapeur ou dans ledit four de grillage ladite quantité de Cl-36 en déchet solide pour l'évacuer via l'utilisation de ladite unité de minéralisation et audit système de solidification.

60. Procédé selon la revendication 1, comprenant en outre les étapes consistant à :
fournir un filtre concentrateur de boue et un système de solidification qui sont raccordés en exploitation audit reformeur à vapeur ou audit four de grillage ;
former dans ledit reformeur à vapeur ou ledit four de grillage des oxydes métalliques, des spinelles métalliques et des formes minérales, lesdits oxydes métalliques comprenant une quantité d'oxydes métalliques insolubles, lesdits spinelles comprenant une quantité de spinelles métalliques insolubles, et lesdites formes minérales comprenant une quantité de formes minérales insolubles ;
concentrer par ledit filtre concentrateur de boue lesdits oxydes métalliques insolubles, lesdits spinelles métalliques insolubles et lesdites formes minérales insolubles ; et
transférer lesdits oxydes métalliques insolubles, lesdits spinelles métalliques et lesdites formes minérales insolubles concentrés vers ledit système de solidification pour les évacuer sous la forme de déchets solides.

61. Procédé selon la revendication 1, comprenant en outre les étapes consistant à :
fournir un filtre concentrateur de boue et une chaudière qui sont raccordés en exploitation audit reformeur à vapeur ou audit four de grillage, ledit filtre concentrateur de boue filtrant l'eau qui est utilisée et formée dans ladite chaudière.

62. Procédé selon la revendication 1, comprenant en outre les étapes consistant à :
fournir un refroidisseur de système de gazéification de graphite qui est raccordé en exploitation audit reformeur à vapeur, ladite étape de chauffage et ladite étape de réaction donnant un gaz de sortie, ledit gaz de sortie comprenant Du C1-36, de la vapeur, des gaz contenant du C-14, de la vapeur d'eau contenant H-3 et des solides particulaires ;
laver ou adsorber par ledit refroidisseur de système de gazéification de graphite ledit C1-36 ;
condenser ladite vapeur et ladite vapeur d'eau contenant H-3 par ledit refroidisseur de système de gazéification de graphite ; et
laver ou retirer lesdits solides particulaires sous la forme d'oxydes métalliques, de spinelles métalliques et de fines de graphites par ledit refroidisseur de système de gazéification de graphite.

63. Procédé selon la revendication 1, comprenant en outre les étapes consistant à :
fournir un four de grillage/gazéificateur/condenseur, dans lequel ladite étape de réaction donne un gaz de sortie qui contient une quantité de C1-36, de vapeur, de gaz contenant du C-14 et de vapeur d'eau contenant H-3 ;
refroidir ledit gaz de sortie par ledit four de grillage/gazéificateur/condenseur ;
adsorber ou laver ledit C1-36 par ledit four de grillage/gazéificateur/condenseur ; et
condenser ladite vapeur et ladite vapeur d'eau contenant H-3 par ledit four de grillage/gazéificateur/condenseur.

64. Procédé selon la revendication 1, dans lequel ledit four de grillage est chauffé par électricité.

65. Procédé selon la revendication 1, comprenant en outre l'étape consistant à introduire des gaz de purge dans ledit four de grillage, dans lequel lesdits gaz de purge comprennent de l'argon, de l'hélium, de l'azote, CO₂, CO, de l'oxygène, des gaz contenant de l'oxygène ou de la vapeur.

66. Procédé selon la revendication 65, dans lequel lesdits gaz de purge s'écoulent à contre-courant par rapport audit graphite.

67. Procédé selon la revendication 1, comprenant en outre l'étape consistant à introduire un cyclage de la pression dans ledit four de grillage.

68. Procédé selon la revendication 1, comprenant en outre l'étape consistant à introduire un cyclage du vide dans ledit four de grillage.

69. Procédé selon la revendication 68, comprenant en outre l'étape consistant à introduire un cyclage de la pression dans ledit four de grillage.

70. Procédé selon la revendication 1, dans lequel ledit four de grillage est exploité à une température comprise entre environ 600 °C et environ 1200 °C.

71. Procédé selon la revendication 1, dans lequel ledit four de grillage est exploité à une température comprise entre 800 °C et environ 1100 °C.

72. Procédé selon la revendication 1, dans lequel ledit agent oxydant comprend de l'oxygène ou un gaz contenant de l'oxygène.

73. Procédé selon la revendication 1, comprenant en outre les étapes consistant à :
fournir un four de grillage/condenseur/laveur et une chaudière qui sont raccordés en exploitation audit four de grillage, ledit graphite comprenant une quantité de H-3 ;
faire réagir ladite quantité de H-3 avec un agent oxydant pour former H₂O contenant H-3 ; et
recycler par ledit four de grillage/condenseur/laveur ledit H₂O contenant H-3 vers ladite chaudière pour concentrer ladite quantité de H-3.

74. Procédé selon la revendication 1, comprenant en outre les étapes consistant à :
fournir un four de grillage/condenseur/laveur qui est raccordé en exploitation audit four de grillage, ledit graphite comprenant une quantité de C1-36 ; et
évacuer par ledit four de grillage/condenseur/laveur ladite quantité de Cl-36.

75. Procédé selon la revendication 1, dans lequel ledit reformeur à vapeur a un mode d'exploitation.

76. Procédé selon la revendication 75, dans lequel ledit mode d'exploitation est fluidisé.

77. Procédé selon la revendication 75, dans lequel ledit mode d'exploitation est un lit fixe sous un lit fluidisé.

78. Procédé selon la revendication 75, dans lequel ledit mode d'exploitation est un lit partiellement jaillissant avec et sans lit fluidisé au-dessus dudit lit partiellement jaillissant.

79. Procédé selon la revendication 75, dans lequel ledit mode d'exploitation est un lit entièrement jaillissant avec et sans lit fluidisé au-dessus dudit lit entièrement jaillissant.

80. Procédé selon la revendication 75, dans lequel ledit mode d'exploitation est un lit fluidisé à courants de recirculation avec gaz de fluidisation avec et sans lit fluidisé au-dessus dudit lit entièrement fluidisé à courants de recirculation.

81. Procédé selon la revendication 1, dans lequel ledit reformeur à vapeur est exploité à une température comprise entre environ 800 °C et environ 1500 °C.

82. Procédé selon la revendication 1, dans lequel ledit reformeur à vapeur est exploité à une température comprise entre environ 1000 °C et environ 1300 °C.

83. Procédé selon la revendication 1, comprenant en outre l'étape consistant à introduire de l'eau dans ledit reformeur à vapeur pour refroidir le contenu dudit reformeur à vapeur.

84. Procédé selon la revendication 1, comprenant en outre l'étape consistant à introduire de l'eau avec un gaz d'atomisation contenant de l'oxygène dans ledit reformeur à vapeur pour refroidir le contenu dudit reformeur à vapeur.

85. Procédé selon la revendication 1, dans lequel ladite étape de chauffage et ladite étape de réaction donnent des fines de graphite, et dans lequel ledit procédé comprend en outre le recyclage vers le reformeur à vapeur desdites fines de graphite, et la gazéification substantielle des dites fines de graphite dans ledit reformeur à vapeur.

86. Procédé selon la revendication 1, dans lequel ladite étape de chauffage et ladite étape de réaction donnent des fines de graphite, et dans lequel ledit procédé comprend en outre le recyclage desdites fines de graphite vers ledit reformeur à vapeur dans une boue à base d'eau, et la gazéification substantielle des dites fines de graphite dans ledit reformeur à vapeur.

87. Procédé selon la revendication 1, dans lequel ladite étape de chauffage et ladite étape de réaction donnent des fines de graphite, et dans lequel ledit procédé comprend en outre le recyclage desdites fines de graphite vers ledit reformeur à vapeur dans une boue à base d'eau et la co-injection de gaz contenant de l'oxygène dans ledit reformeur à vapeur, et la gazéification substantielle des dites fines de graphite.

88. Procédé selon la revendication 1, dans lequel ladite étape de chauffage et ladite étape de réaction donnent des fines de graphite, et dans lequel ledit procédé comprend en outre le recyclage desdites fines de graphite vers ledit reformeur à vapeur dans une boue à base d'eau et la co-injection de gaz contenant de l'oxygène pour gazéifier substantiellement lesdites fines de graphite dans ledit reformeur à vapeur, et l'ajout d'eau simultanément à ladite étape de co-injection pour refroidir le contenu dudit reformeur à vapeur, ladite eau étant atomisée par ledit gaz contenant de l'oxygène.

89. Procédé selon la revendication 1, dans lequel ladite étape de chauffage et ladite étape de réaction donnent des fines de graphite, et dans lequel ledit procédé comprend en outre la fourniture d'un système de transfert pneumatique à sec, le recyclage desdites fines de graphite dans ledit reformeur à vapeur avec ledit système de transfert pneumatique à sec et la gazéification substantielle desdites fines de graphite.

90. Procédé selon la revendication 1, dans lequel ledit agent de reformage et ledit agent oxydant sont un gaz de fluidisation.

91. Procédé selon la revendication 1, dans lequel ledit agent de reformage et ledit agent oxydant sont un gaz contenant de l'eau et de l'oxygène.

92. Procédé selon la revendication 1, dans lequel ledit agent de reformage est un gaz de fluidisation et dans lequel ledit agent oxydant est un gaz contenant de l'eau.

93. Procédé selon la revendication 1, dans lequel ledit agent de reformage est un gaz de fluidisation et dans lequel ledit agent oxydant est un gaz contenant de l'eau et de l'oxygène.

94. Procédé selon la revendication 1, dans lequel ledit agent de reformage est un gaz de fluidisation et dans lequel ledit agent oxydant est un gaz contenant de l'oxygène.

95. Procédé selon la revendication 1, dans lequel ledit reformeur à vapeur contient un lit de graphite, dans lequel ladite étape de réaction donne la formation d'hydrogène et dans lequel ladite étape de réaction comprend en outre la réaction dudit hydrogène et dudit oxyde de carbone avec un agent oxydant pour former de l'eau et du dioxyde de carbone, et dans lequel ladite étape de réaction se produit sur la portion supérieure dudit lit.

96. Procédé selon la revendication 1, dans lequel ledit reformeur à vapeur comprend un lit de graphite, dans lequel ladite étape de réaction donne la formation d'hydrogène et dans lequel ladite étape de réaction comprend en outre la réaction dudit hydrogène et dudit oxyde de carbone avec un agent oxydant pour former de l'eau et du dioxyde de carbone, et dans lequel ladite étape de réaction se produit au-dessus dudit lit.

97. Procédé selon la revendication 1, comprenant en outre l'étape consistant à fournir un moyen de calibrage du graphite qui est raccordé en exploitation audit reformeur à vapeur.

98. Procédé selon la revendication 1, dans lequel ledit four de grillage fonctionne indépendamment dudit reformeur à vapeur.

99. Procédé selon la revendication 1, dans lequel ledit graphite comprend une quantité d'hydrogène, et dans lequel ledit procédé comprend en outre la réaction de ladite quantité d'hydrogène avec un agent oxydant pour former de l'eau dans ledit reformeur à vapeur, et le refroidissement de ladite eau en injectant de l'eau supplémentaire dans ledit reformeur à vapeur.

100. Procédé selon la revendication 1, comprenant en outre le refroidissement du contenu dudit reformeur à vapeur par ajout d'eau et d'un gaz d'atomisation contenant de l'oxygène.
